



US012281441B2

(12) **United States Patent**  
**Flynn et al.**

(10) **Patent No.:** **US 12,281,441 B2**  
(b4) **Date of Patent:** **Apr. 22, 2025**

(54) **METHODS AND SYSTEMS FOR FORMING COMPOSITE FIBERS**

(71) Applicant: **EVRNU, SPC**, Seattle, WA (US)

(72) Inventors: **Stacy Flynn**, Seattle, WA (US);  
**Christopher Stanev**, Rutherford, NJ (US)

(73) Assignee: **EVRNU, SPC**, Seattle, WA (US)

(\*) Notice: Subject to any disclaimer, the term of this patent is extended or adjusted under 35 U.S.C. 154(b) by 511 days.

(21) Appl. No.: **17/088,833**

(22) Filed: **Nov. 4, 2020**

(65) **Prior Publication Data**

US 2021/0054567 A1 Feb. 25, 2021

**Related U.S. Application Data**

(60) Division of application No. 15/491,816, filed on Apr. 19, 2017, now abandoned, which is a continuation-in-part of application No. PCT/US2016/044325, filed on Jul. 27, 2016, and a continuation-in-part of application No. 14/811,723, filed on Jul. 28, 2015, now abandoned, said application No. PCT/US2016/044325 is a continuation-in-part of application No. 14/811,723, filed on Jul. 28, 2015, now abandoned, which is a continuation-in-part of application No. 14/255,886, filed on Apr. 17, 2014, now abandoned.

(60) Provisional application No. 62/325,383, filed on Apr. 20, 2016, provisional application No. 62/214,708, filed on Sep. 4, 2015, provisional application No. 62/198,077, filed on Jul. 28, 2015, provisional application No. 61/812,931, filed on Apr. 17, 2013.

(51) **Int. Cl.**

**D21H 13/08** (2006.01)  
**D21H 17/00** (2006.01)  
**D21H 17/63** (2006.01)

(52) **U.S. Cl.**

CPC ..... **D21H 13/08** (2013.01); **D21H 17/005** (2013.01); **D21H 17/74** (2013.01); **D21H 17/63** (2013.01)

(58) **Field of Classification Search**

CPC ..... D21H 13/08; D21H 17/005; D21H 17/74; D21H 17/63

See application file for complete search history.

(56) **References Cited**

U.S. PATENT DOCUMENTS

2,039,307 A 5/1936 Dreyfus  
2,047,136 A 7/1936 Doyle

|              |          |                    |
|--------------|----------|--------------------|
| 2,064,473 A  | 12/1936  | Holdsworth         |
| 2,100,830 A  | 11/1937  | Altheide           |
| 2,307,863 A  | 1/1943   | Soukup             |
| 2,337,458 A  | 12/1943  | Edson              |
| 3,057,772 A  | 10/1962  | Magill, Jr.        |
| 3,320,066 A  | 5/1967   | Garth              |
| 3,344,016 A  | 9/1967   | Moggio et al.      |
| 3,895,089 A  | 7/1975   | Goyal              |
| 4,012,281 A  | 3/1977   | Mayer et al.       |
| 4,018,646 A  | 4/1977   | Ruffo et al.       |
| 4,081,582 A  | 3/1978   | Butterworth et al. |
| 4,409,384 A  | 10/1983  | Lindsey            |
| 4,426,516 A  | 1/1984   | Kuriki et al.      |
| 4,634,470 A  | * 1/1987 | Kamide             |
|              |          | C08L 1/02          |
|              |          | 106/166.01         |
| 4,963,230 A  | 10/1990  | Kawase et al.      |
| 5,009,747 A  | 4/1991   | Viazmensky et al.  |
| 5,106,457 A  | 4/1992   | Manning            |
| 5,208,004 A  | 5/1993   | Myerson et al.     |
| 5,238,534 A  | 8/1993   | Manning et al.     |
| 5,281,269 A  | 1/1994   | Ganci et al.       |
| 5,342,854 A  | 8/1994   | Serad              |
| 5,415,738 A  | 5/1995   | Mehta et al.       |
| 5,601,767 A  | 2/1997   | Firgo              |
| 5,609,676 A  | 3/1997   | von der Eltz       |
| 5,853,493 A  | 12/1998  | Skelton et al.     |
| 5,868,985 A  | 2/1999   | Frischmann         |
| 5,980,746 A  | 11/1999  | Gelman et al.      |
| 6,010,542 A  | 1/2000   | DeYoung et al.     |
| 6,210,801 B1 | 4/2001   | Luo                |

(Continued)

FOREIGN PATENT DOCUMENTS

|    |           |        |
|----|-----------|--------|
| CN | 103060844 | 4/2013 |
| CN | 112709092 | 6/2022 |

(Continued)

OTHER PUBLICATIONS

Negulescu et al. Recycling Cotton from Cotton/Polyester Fabrics. Textile Chemist and Colorist, vol. 30. No. 6, Jun. 1998, pp. 31-35.\*

(Continued)

*Primary Examiner* — Amina S Khan

(74) *Attorney, Agent, or Firm* — Summit Patents PC

(57)

**ABSTRACT**

Methods and systems of the present invention use cellulose-containing materials, which may include post-consumer waste garments, scrap fabric and/or various biomass materials as a raw feed material to produce isolated cellulose molecules that can be used in the textile and apparel industries, and in other industries. A multi-stage process is provided, in which cellulose-containing feed material is subjected to one or more pretreatment stages, followed by a dissolution treatment and isolation of cellulose molecules. Isolated cellulose molecules may be used in a variety of downstream applications. Methods and systems for carbonizing precursor fibers to produce carbonized fibers having desired properties and three-dimensional configurations are provided.

| (56)                  | References Cited |                      | WO                                                                                                                                                                                                                                                                                             | WO 01/86042  | *                                                                                                                                                                                               | 11/2001 | ..... | D01F 2/00 |  |  |
|-----------------------|------------------|----------------------|------------------------------------------------------------------------------------------------------------------------------------------------------------------------------------------------------------------------------------------------------------------------------------------------|--------------|-------------------------------------------------------------------------------------------------------------------------------------------------------------------------------------------------|---------|-------|-----------|--|--|
| U.S. PATENT DOCUMENTS |                  |                      |                                                                                                                                                                                                                                                                                                |              |                                                                                                                                                                                                 |         |       |           |  |  |
| 6,214,976 B1          | 4/2001           | Watanabe et al.      | WO                                                                                                                                                                                                                                                                                             | 2001096402   | 12/2001                                                                                                                                                                                         |         |       |           |  |  |
| 6,235,392 B1          | 5/2001           | Luo et al.           | WO                                                                                                                                                                                                                                                                                             | WO 01/96402  | *                                                                                                                                                                                               | 12/2001 | ..... | C08B 1/00 |  |  |
| 6,302,997 B1          | 10/2001          | Hurter               | WO                                                                                                                                                                                                                                                                                             | 2011077446   | 6/2011                                                                                                                                                                                          |         |       |           |  |  |
| 6,344,077 B1          | 2/2002           | Hong                 | WO                                                                                                                                                                                                                                                                                             | 2012156441   | 11/2012                                                                                                                                                                                         |         |       |           |  |  |
| 6,607,637 B1          | 8/2003           | Vinson et al.        | WO                                                                                                                                                                                                                                                                                             | 2013124265   | 8/2013                                                                                                                                                                                          |         |       |           |  |  |
| 6,861,380 B2          | 3/2005           | Garnier et al.       | WO                                                                                                                                                                                                                                                                                             | 2013145236   | 10/2013                                                                                                                                                                                         |         |       |           |  |  |
| 7,828,936 B2          | 11/2010          | Luo et al.           | WO                                                                                                                                                                                                                                                                                             | 2014045062   | 3/2014                                                                                                                                                                                          |         |       |           |  |  |
| 7,981,337 B2          | 7/2011           | Zhang et al.         | WO                                                                                                                                                                                                                                                                                             | 2014060651   | 4/2014                                                                                                                                                                                          |         |       |           |  |  |
| 8,361,278 B2          | 1/2013           | Fike et al.          | WO                                                                                                                                                                                                                                                                                             | WO2014081291 | 5/2014                                                                                                                                                                                          |         |       |           |  |  |
| 8,454,799 B2          | 6/2013           | Jehn-Rendu et al.    | WO                                                                                                                                                                                                                                                                                             | 2014149024   | 9/2014                                                                                                                                                                                          |         |       |           |  |  |
| 8,827,192 B2          | 9/2014           | Innerlohinger et al. | WO                                                                                                                                                                                                                                                                                             | 2014162062   | 10/2014                                                                                                                                                                                         |         |       |           |  |  |
| 8,962,821 B2          | 2/2015           | Zhang et al.         | WO                                                                                                                                                                                                                                                                                             | 2015018464   | 2/2015                                                                                                                                                                                          |         |       |           |  |  |
| 9,121,137 B2          | 9/2015           | Viazmensky et al.    | WO                                                                                                                                                                                                                                                                                             | 2016012755   | 1/2016                                                                                                                                                                                          |         |       |           |  |  |
| 9,145,645 B2          | 9/2015           | Reed et al.          | WO                                                                                                                                                                                                                                                                                             | 2016110836   | 7/2016                                                                                                                                                                                          |         |       |           |  |  |
| 9,315,840 B2          | 4/2016           | Genta                | WO                                                                                                                                                                                                                                                                                             | 2017135816   | 8/2017                                                                                                                                                                                          |         |       |           |  |  |
| 9,611,371 B2          | 4/2017           | Walker               | OTHER PUBLICATIONS                                                                                                                                                                                                                                                                             |              |                                                                                                                                                                                                 |         |       |           |  |  |
| 10,065,379 B2         | 9/2018           | Fretz                | Communication pursuant to Article 94(3) EPC mailed May 31, 2022, EP Application No. 16831317.9.                                                                                                                                                                                                |              |                                                                                                                                                                                                 |         |       |           |  |  |
| 10,704,199 B2         | 7/2020           | Henaff et al.        | Negulesca et al., "Recycling Cotton from Cotoon/Polyester Fabrics", Textile Chemist and Colorist, Jun. 1998, pp. 31-35.                                                                                                                                                                        |              |                                                                                                                                                                                                 |         |       |           |  |  |
| 11,034,817 B2         | 6/2021           | Flynn et al.         | Anderson, Kim Ph.D., "Dyeing Textiles with Supercritical Carbon Dioxide: A Non-Aqueous Dyeing System", www.techexchange.com, p. 14, Jan. 2009.                                                                                                                                                 |              |                                                                                                                                                                                                 |         |       |           |  |  |
| 11,441,267 B2         | 9/2022           | Mitchell et al.      | (Anonymous), "Synthesis of Schweizer's Reagent then Precipitation of Rayon by Acidification by Disulfideprotein", D Science Madness Discussion Board, Special Topics, Prepublication, www.sciencemadness.org (Jul. 3, 2012).                                                                   |              |                                                                                                                                                                                                 |         |       |           |  |  |
| 2003/0056916 A1       | 3/2003           | Horenziak et al.     | Hou, Aigin et al., "Using supercritical carbon dioxide as solvent to replace water in polyethylene terephthalate (PET) fabric dyeing procedures", National Engineering Research Center for Dyeing and Finishing of Textiles, Donghua University, Shanghai 201620, China (Jul. 2010). Abstract. |              |                                                                                                                                                                                                 |         |       |           |  |  |
| 2004/0126555 A1*      | 7/2004           | Hartmann .....       | D04H 1/4383                                                                                                                                                                                                                                                                                    | 428/296.7    | Pacific Northwest Pollution Prevention Resource Center, "Supercritical Carbon-Dioxide Cleaning Technology Review," http://www.pprc.org/pubs/techreviews/co2/co2intro.html, pp. 1-2 (Jul. 1996). |         |       |           |  |  |
| 2005/0234229 A1       | 10/2005          | Loth et al.          | Schamotia, Justin "Cotton Recycling Process", eHow.com, http://www.chow.com/prinUinfo_8685561_cotton-recycling-process.html.                                                                                                                                                                   |              |                                                                                                                                                                                                 |         |       |           |  |  |
| 2006/0213839 A1       | 9/2006           | Huang et al.         | Van Roosmalen, M.J.E. et al., "Dry-cleaning with high-pressure carbon dioxide—the influence of mechanical action on washing results", Journal of Supercritical Fluids, vol. 27, No. 97, p. 108 (Sep. 2002). Abstract.                                                                          |              |                                                                                                                                                                                                 |         |       |           |  |  |
| 2008/0135193 A1       | 6/2008           | Kokko                | Dadi, AP et al., "Enhancement of Cellulose Saccharification Kinetics Using an Ionic Liquid Pretreatment Step, Biotechnology and Bioengineering", Aug. 17, 2006, p. 905, col. 2, paragraph 1 to p. 906, col. 1, paragraph 3.                                                                    |              |                                                                                                                                                                                                 |         |       |           |  |  |
| 2008/0275231 A1       | 11/2008          | Zhang et al.         | Wang, "Cellulose Fiber Dissolution in Sodium Hydroxide Solution at Low Temperature: Dissolution Kinetics and Solubility Improvement", Georgia Institute of Technology, Dec. 2008.                                                                                                              |              |                                                                                                                                                                                                 |         |       |           |  |  |
| 2010/0162542 A1       | 7/2010           | Luo et al.           | Wahlstrom, "Enzymatic Hydrolysis of Cellulose in Aqueous Ionic Liquids", VTT Technical Research Centre of Finland, Feb. 21, 2014.                                                                                                                                                              |              |                                                                                                                                                                                                 |         |       |           |  |  |
| 2010/0200184 A1       | 8/2010           | Levit et al.         | Okimori et al., "Potential of Carbon Sequestration by Carbonizing Wood Residue from Industrial Tree Plantation as a Clean Development Mechanism Project in the Kyoto Mechanism", Energy with Agricultural Carbon Utilization Symposium, Georgia.                                               |              |                                                                                                                                                                                                 |         |       |           |  |  |
| 2010/0298555 A1       | 11/2010          | Okutsu               | Peterson, "Towards Recycling of Textile Fibers", Chalmers University of Technology, 2015.                                                                                                                                                                                                      |              |                                                                                                                                                                                                 |         |       |           |  |  |
| 2011/0094691 A1       | 4/2011           | Nunn                 | De Silva et al., "The Separation & Utilization of Polyester/Cotton Blends", 17th Australian Cotton Conference.                                                                                                                                                                                 |              |                                                                                                                                                                                                 |         |       |           |  |  |
| 2011/0201096 A1       | 8/2011           | Streffer             | Akato, "Pretreatment and Pyrolysis of Rayon-based Precursor for Carbon Fibers", University of Tennessee, Knoxville, 2012.                                                                                                                                                                      |              |                                                                                                                                                                                                 |         |       |           |  |  |
| 2012/0000621 A1       | 1/2012           | Stigsson             | Li et al., "A Mechanism Study on Preparation of rayon Based Carbon Fibers with (NH4)2SO4/NH3Cl/organosilicon Composite Catalyst System", Composites Science and Technology, 2007.                                                                                                              |              |                                                                                                                                                                                                 |         |       |           |  |  |
| 2012/0028116 A1       | 2/2012           | Choi et al.          | Ma et al., "Mechanical, Microstructure and Surface Characterizations of Carbon Fibers Prepared from Cellulose after Liquefying and Curing", Tianjin University of Science and Technology, Dec. 20, 2013.                                                                                       |              |                                                                                                                                                                                                 |         |       |           |  |  |
| 2012/0241669 A1       | 9/2012           | Jiang et al.         |                                                                                                                                                                                                                                                                                                |              |                                                                                                                                                                                                 |         |       |           |  |  |
| 2013/0189474 A1       | 7/2013           | Kroner et al.        |                                                                                                                                                                                                                                                                                                |              |                                                                                                                                                                                                 |         |       |           |  |  |
| 2014/0205830 A1       | 7/2014           | Malinowsky et al.    |                                                                                                                                                                                                                                                                                                |              |                                                                                                                                                                                                 |         |       |           |  |  |
| 2014/0308862 A1       | 10/2014          | Heinzman et al.      |                                                                                                                                                                                                                                                                                                |              |                                                                                                                                                                                                 |         |       |           |  |  |
| 2014/0315461 A1       | 10/2014          | Schachtnet et al.    |                                                                                                                                                                                                                                                                                                |              |                                                                                                                                                                                                 |         |       |           |  |  |
| 2014/0318415 A1       | 10/2014          | Innerlohinger et al. |                                                                                                                                                                                                                                                                                                |              |                                                                                                                                                                                                 |         |       |           |  |  |
| 2014/0343270 A1       | 11/2014          | Lindstrom et al.     |                                                                                                                                                                                                                                                                                                |              |                                                                                                                                                                                                 |         |       |           |  |  |
| 2014/0364538 A1       | 12/2014          | Baney et al.         |                                                                                                                                                                                                                                                                                                |              |                                                                                                                                                                                                 |         |       |           |  |  |
| 2015/0007952 A1       | 1/2015           | Möderl et al.        |                                                                                                                                                                                                                                                                                                |              |                                                                                                                                                                                                 |         |       |           |  |  |
| 2015/0159302 A1       | 6/2015           | Leitner et al.       |                                                                                                                                                                                                                                                                                                |              |                                                                                                                                                                                                 |         |       |           |  |  |
| 2015/0330029 A1       | 11/2015          | Ramaratnam et al.    |                                                                                                                                                                                                                                                                                                |              |                                                                                                                                                                                                 |         |       |           |  |  |
| 2016/0040360 A1       | 2/2016           | Li et al.            |                                                                                                                                                                                                                                                                                                |              |                                                                                                                                                                                                 |         |       |           |  |  |
| 2016/0362841 A1       | 12/2016          | Fretz                |                                                                                                                                                                                                                                                                                                |              |                                                                                                                                                                                                 |         |       |           |  |  |
| 2016/0369456 A1       | 12/2016          | Flynn et al.         |                                                                                                                                                                                                                                                                                                |              |                                                                                                                                                                                                 |         |       |           |  |  |
| 2017/0152633 A1       | 6/2017           | Hagihara et al.      |                                                                                                                                                                                                                                                                                                |              |                                                                                                                                                                                                 |         |       |           |  |  |
| 2017/0218162 A1       | 8/2017           | Walker               |                                                                                                                                                                                                                                                                                                |              |                                                                                                                                                                                                 |         |       |           |  |  |
| 2017/0282523 A1       | 10/2017          | Cabell et al.        |                                                                                                                                                                                                                                                                                                |              |                                                                                                                                                                                                 |         |       |           |  |  |
| 2017/0328012 A1       | 11/2017          | Lee et al.           |                                                                                                                                                                                                                                                                                                |              |                                                                                                                                                                                                 |         |       |           |  |  |
| 2018/0051416 A1       | 2/2018           | Lu et al.            |                                                                                                                                                                                                                                                                                                |              |                                                                                                                                                                                                 |         |       |           |  |  |
| 2018/0018377 A1       | 7/2018           | Ziegenbein           |                                                                                                                                                                                                                                                                                                |              |                                                                                                                                                                                                 |         |       |           |  |  |
| 2018/0215893 A1       | 8/2018           | Flynn et al.         |                                                                                                                                                                                                                                                                                                |              |                                                                                                                                                                                                 |         |       |           |  |  |
| 2018/0266054 A1       | 9/2018           | Henaff et al.        |                                                                                                                                                                                                                                                                                                |              |                                                                                                                                                                                                 |         |       |           |  |  |
| 2018/0274174 A1       | 9/2018           | Tanaka et al.        |                                                                                                                                                                                                                                                                                                |              |                                                                                                                                                                                                 |         |       |           |  |  |
| 2018/0347110 A1       | 12/2018          | Hart et al.          |                                                                                                                                                                                                                                                                                                |              |                                                                                                                                                                                                 |         |       |           |  |  |
| 2019/0257032 A1       | 8/2019           | Kawahara et al.      |                                                                                                                                                                                                                                                                                                |              |                                                                                                                                                                                                 |         |       |           |  |  |
| 2021/0054567 A1       | 2/2021           | Flynn et al.         |                                                                                                                                                                                                                                                                                                |              |                                                                                                                                                                                                 |         |       |           |  |  |
| 2021/0246581 A1       | 8/2021           | Flynn et al.         |                                                                                                                                                                                                                                                                                                |              |                                                                                                                                                                                                 |         |       |           |  |  |
| 2021/0340350 A1       | 11/2021          | Flynn et al.         |                                                                                                                                                                                                                                                                                                |              |                                                                                                                                                                                                 |         |       |           |  |  |
| 2021/0381166 A1       | 12/2021          | Flynn et al.         |                                                                                                                                                                                                                                                                                                |              |                                                                                                                                                                                                 |         |       |           |  |  |
| 2022/0325479 A1       | 10/2022          | Shi et al.           |                                                                                                                                                                                                                                                                                                |              |                                                                                                                                                                                                 |         |       |           |  |  |

## FOREIGN PATENT DOCUMENTS

|    |            |        |
|----|------------|--------|
| EP | 0743393    | 5/1996 |
| FI | 92133 B    | 6/1994 |
| GB | 1473882    | 5/1977 |
| JP | 2000192393 | 7/2000 |
| JP | 2002105894 | 4/2002 |
| TW | 201529648  | 8/2015 |
| WO | 9720102    | 6/1997 |

(56)

**References Cited****OTHER PUBLICATIONS**

- Park et al., "Precursors and Manufacturing of Carbon Fibers", Carbon Fibers, 2015.
- Bhat et al., "Recent Developments on Carbon Fibers from Rayon-Based Precursors", The University of Tennessee, Knoxville.
- Holding, "Ionic Liquids and Electrolytes for Cellulose Dissolution", University of Helsinki, 2016.
- Seger et al., "Solution behaviour of cellulose and amylose in iron-sodiumtartrate (FeTNa)", Carbohydrate polymers, 31 (1996) 105-112.
- Saxen et al., "Viscometric Determination of molecular weight of cellulose pulps in zinc ethylenediamine solution", Journal of Applied Polymer Science, 1963, vol. 7, Issue 1; Abstract.
- Shenouda et al., "Swelling of coton in zincoxen", European Polymer Journal, 1975, vol. 12, Issue 5. Abstract.

Harzallah et al, "Physical and Mechanical Properties of Cotton Fibers: Single-fiber Failure", Textile Research Journal, 2009, vol. 80, Issue 11. Abstract.

Landon et al., "Facile Green Synthesis of Large Single Crystal Cooper Micro and Nanoparticles with Ascorbic Acid and Gum Arabic", Open Journal of Applied Sciences, 2013, 3 332-336.

International Search Report and the Written Opinion of the International Searching Authority, Nov. 15, 2016, PCT/US2016/044325. International Preliminary Report on Patentability, issued Jan. 30, 2018, in International Application No. PCT/US2016-044325, date of filing Jul. 27, 2016.

Beckman, "Supercritical and near-critical CO<sub>2</sub> in green chemical synthesis and processing", Journal of Supercritical Fluids, vol. 28, pp. 121-191, 2004.

Hsieh, Y.L., "Chemical structure and properties of cotton" Cotton: Science and technology, (2007) 3-34.

Shaw et al in "Rayon as Paper-Making Material" Bureau of Standards Journal of Research, vol. 4, pp. 203-211. (Year: 1929).

\* cited by examiner



FIG. 1



FIG. 2



FIG. 3



FIG. 4



FIG. 5

**FIG. 6**



FIG. 7



FIG. 8

**FIG. 9**

**FIG. 10**



***FIG. 11A***

***FIG. 11B***



***FIG. 11C***



FIG. 12



FIG. 13



**FIG. 14A**



**FIG. 14B**

## 1

METHODS AND SYSTEMS FOR FORMING  
COMPOSITE FIBERS

## REFERENCE TO RELATED APPLICATIONS

This application is a divisional of pending U.S. patent application Ser. No. 15/491,816, filed Apr. 19, 2017, which is a continuation-in-part of pending U.S. patent application Ser. No. 14/811,723, filed Jul. 28, 2015, which is a continuation-in-part of U.S. patent application Ser. No. 14/255,886, filed Apr. 17, 2014, abandoned, which claims the benefit of U.S. Patent Application No. 61/812,931, filed Apr. 17, 2013. Pending U.S. patent application Ser. No. 15/491,816 is also a continuation-in-part of pending PCT Int'l Application No. PCT/US16/44325, filed Jul. 27, 2016, which is a continuation-in-part of U.S. patent application Ser. No. 14/811,723, filed Jul. 28, 2015 and claims the benefit of U.S. Patent Application No. 62/198,077, filed Jul. 28, 2015 and to U.S. Patent Application No. 62/214,708, filed Sep. 4, 2015. Pending U.S. patent application Ser. No. 15/491,816 also claims the benefit of U.S. Patent Application No. 62/325,383, filed Apr. 20, 2016. These applications are incorporated herein by reference in their entireties.

## FIELD

The present disclosure relates to methods and systems for processing cellulose-containing materials such as textiles, including textile garments (used and un-used) and scraps, biomass, wood pulp, and the like and for isolating cellulose molecules for use in a variety of downstream applications. In particular applications, the present disclosure relates to methods and systems for treatment of cellulose-containing materials to isolate cellulose molecules and to produce regenerated polymers, fibers, and/or fabrics from the isolated cellulose molecules. In additional aspects, methods for carbonizing fibers and carbonized fibers having pre-determined cross-sections and three-dimensional configurations are disclosed. Recycling and regeneration of textiles is described in detail and provides significant social, environmental and economic benefits.

## BACKGROUND

Global sales of apparel are estimated to have exceeded \$1 trillion in 2011, and some estimate that over 85% of the garments purchased are discarded in a landfill within one year. This cycle wastes valuable materials and the considerable resources required to produce them, and it exacerbates waste disposal issues.

Cotton clothing is estimated to represent about 35% of the total apparel market. Cotton fibers are composed of cellulose, a naturally occurring polymer found in all plants, wood, and natural fibers. Cotton fibers are harvested from cotton plants and consist of long, interwoven chains of cellulose polymers. These fibers are spun into thread or yarn, dyed, and ultimately woven, knit, and assembled into textiles. Natural fibers, including cotton, have a generally high and variable raw material cost due, in part, to natural disasters and climate unpredictability, regional socio-economic and political instability, human rights issues, and resource requirements.

Growing and harvesting cotton fibers is resource-intensive. It is estimated, for example, that over 700 gallons of water are required to grow enough cotton to produce one pound of fiber. Growing cotton frequently involves heavy pesticide use, significant land resources, and produces sig-

## 2

nificant levels of heat-trapping gases. Considerably more land is required for growing organic cotton than for growing "conventional" cotton. With demand for agricultural land use increasing and fresh water supplies decreasing, the cost of producing natural cotton is increasing. At some point, the current scale of cotton production may become unprofitable and unsustainable.

Cotton has been recycled to provide raw material for paper pulping plants. Re-processing methods that convert used cotton into rags, mattress ticking, seat stuffing, insulating materials, and the like are also available, but these processing methods have been adopted in limited applications because the value of the converted material is relatively low.

In contrast to cotton, which is a natural fiber, rayon fibers are manufactured from wood pulp using the viscose process. In this process, purified cellulose is solubilized and then converted or regenerated into cellulose fiber. This process requires steeping, pressing, shredding, aging, xanthation, dissolving, ripening, filtering, degassing, spinning, drawing and washing. This process is time sensitive, requires multiple chemical treatments, produces lignin and other waste from unusable wood material and is, at best, a semi-continuous manufacturing process.

The present disclosure is directed to providing systems and methods for processing cellulose-containing feedstocks, such as recycled fabric, fabric scraps and other cellulose containing materials, many of which would otherwise be wasted or used to produce low value products, to isolate their constituent cellulosic polymeric structures. The polymeric cellulosic structures are then used in industrial processes such as fabric production. Implementation of the disclosed processing schemes with a variety of garment/fabric feedstock materials may produce regenerated fibers and textile products having improved and/or customize-able properties using processes having low environmental impacts.

## SUMMARY

Methods and systems of the present disclosure relate to processing of cellulose-containing materials including, for example, postconsumer cellulosic waste, cellulose-containing textiles and garments (e.g., recycled or used or waste textiles and garments), virgin cotton, wood pulp, biomass, and the like, to produce isolated cellulose polymers for use in downstream processing applications. In some embodiments, cellulose-containing materials used as raw feed material for processing comprise discarded garments and/or scrap fabric materials, and processing produces isolated cellulose polymers that can be further processed and extruded to provide regenerated fibers having improved and/or customize-able properties for use in textile industries or for other purposes.

A multi-stage process is described, incorporating one or more pretreatment stages providing removal of contaminants and preparation of cellulosic materials, followed by cellulose dissolution and/or molecular separation of cellulose polymers. In some embodiments, the pretreatment and cellulose dissolving processes may be carried out in a continuous, semi-continuous or batch system. In some embodiments, the pretreatment and cellulose dissolving processes may be carried out in one or more closed reaction vessel(s), and processing reagents may be recovered and re-used or processed for other uses.

Numerous pretreatment processing stages are described and may be used alone or in combination to remove non-

cellulosic constituents of the feed and prepare cellulosic components for cellulose dissolution. Pretreatment is followed by at least one cellulose dissolution stage that promotes the molecular separation and isolation of cellulose polymers, such as by disrupting intermolecular hydrogen bonds. In some embodiments, cellulosic polymers isolated during the dissolution stage(s) are substantially thermoplastic and are moldable when energy (e.g., heat below the char point) is introduced to the system.

Isolated cellulose polymers produced using the processes described herein may be used in a variety of downstream applications, as described in more detail below and, in some embodiments, may be extruded to form regenerated cellulosic fibers. In some aspects, isolated cellulose polymers may be re-generated to provide longer chain polymers and fibers (or polymers and fibers having other desirable characteristics different from the characteristics of the cellulose-containing feedstock) that are useful in various industrial processes, including textile production. In addition to employing raw feedstock materials that are typically discarded (wasted, at a cost), processing steps having generally low environmental impacts are preferred.

Isolated cellulose polymers (and other precursor polymers) may be extruded and processed in accordance with methods described below to provide carbonized fibers. Carbonized fibers may be produced from a variety of precursors, including fibers generated from post-consumer waste textile feedstocks. Fibers having desired cross-sectional sizes and configurations may be carbonized under conditions that impart three-dimensional configurations to the carbonized fibers. Carbon fibers can be coiled or formed in desired three-dimensional configurations to engineer desired mechanical properties. Such carbonized fibers have superior properties, such as superior insulating properties and are light weight and may be further treated to impart desired surface, structural or chemical properties. Such carbonized fibers are generally provided as microstructures that may be integrated in matrixes or fabrics to provide cushioning, stretch and elastic properties.

In one aspect, methods and systems of the present disclosure provide a closed-loop garment recycling process that transforms reclaimed garments and textiles into high-quality, bio-based fiber for use in creating new textiles, apparel, and other fiber-based products. Used and waste garment collection, sorting, transport and processing may all be involved as part of a closed loop process. Retail enterprises (and others) may serve as collection stations and may offer incentives, rewards, or the like for donations. Further garment processing may take place at the donation site or at one or more remote sites. Cotton, cotton-like regenerated fabrics, rayon and other fibers may be produced using the reclaimed garments and textiles.

#### BRIEF DESCRIPTION OF THE DRAWINGS

FIG. 1 illustrates an exemplary schematic flow diagram outlining process steps as disclosed herein for converting cellulose-containing materials to liquefied cellulose suitable for use in a variety of downstream applications.

FIG. 2 illustrates an exemplary schematic flow diagram outlining process steps as disclosed herein for converting cellulose-containing materials to regenerated cellulosic fiber and incorporating one or more of a variety of pretreatments.

FIG. 3 illustrates an exemplary schematic flow diagram outlining process steps as disclosed herein for converting cellulose-containing materials to regenerated cellulosic fiber

incorporating a high temperature aqueous or supercritical carbon dioxide pretreatment step and incorporating optional additional treatment steps.

FIG. 4 illustrates an exemplary schematic flow diagram outlining process steps as disclosed herein for converting cellulose-containing materials to regenerated cellulosic fiber incorporating a combination of pretreatment steps.

FIG. 5 illustrates an exemplary schematic flow diagram outlining process steps as disclosed herein for converting cellulose-containing materials to regenerated cellulosic fiber incorporating another combination of pretreatment steps.

FIG. 6 illustrates an exemplary schematic flow diagram outlining process steps as disclosed herein for converting cellulose-containing materials to regenerated cellulosic fiber incorporating another combination of pretreatment steps.

FIG. 7 illustrates an exemplary schematic flow diagram outlining process steps as disclosed herein for converting cellulose-containing materials to regenerated cellulosic fiber incorporating yet another combination of pretreatment steps.

FIG. 8 illustrates an exemplary schematic flow diagram outlining process steps as disclosed herein for processing blended textile input to produce liquefied cellulosic and polymeric output.

FIG. 9 illustrates an exemplary schematic flow diagram illustrating additional features of dissolving stage.

FIG. 10 illustrates an exemplary schematic flow diagram illustrating dissolving solvents and the production of regenerated cellulosic fiber.

FIG. 11A shows a magnified image of a regenerated cellulosic fiber produced as described herein; FIG. 11B shows a magnified image of a premium long-staple cotton fiber as tested in Harzallah, Benzina & Drean, 2009; and FIG. 11C shows an enlarged, cross-sectional view of a regenerated cellulosic fiber produced as described herein.

FIG. 12 illustrates an exemplary schematic flow diagram outlining process steps as disclosed herein for converting blended textile input comprising predominantly cellulose-containing materials to liquefied cellulose and liquefied polyester suitable for use in a variety of downstream applications.

FIG. 13 illustrates an exemplary schematic flow diagram outlining process steps as disclosed herein for converting blended textile input comprising predominantly polyester-containing materials to liquefied polyester and liquefied cellulose suitable for use in a variety of downstream applications.

FIGS. 14A and 14B schematically illustrate the processing of liquefied cellulose and liquefied polyester, respectively, to produce regenerated cellulosic fiber and regenerated polyester fiber, respectively.

It will be understood that the appended drawings present many alternatives and various specific embodiments, and that there are many variations and combinations of processing steps, as well as additional aspects of systems and methods of the present invention. Specific process design features may be modified and used in different combinations, for example, for use in various intended applications and environments.

#### DETAILED DESCRIPTION

In one aspect, systems and methods disclosed herein process cellulose-containing materials to produce isolated cellulosic polymers suitable for use in downstream processing and a variety of downstream applications and production pathways. Cellulose-containing materials that are useful as raw materials for this process include a wide range of

materials, such as cellulose-containing postconsumer waste, biomass materials and pulp (e.g., wood pulp), cotton and cotton-containing materials, and the like, including unworn or worn and discarded cotton and cotton-containing apparel, as well as scrap cotton fiber and fabric. The cellulose-containing feedstock undergoes at least one pretreatment stage (and optionally multiple pretreatment stages) and at least one dissolution stage to produce isolated cellulose molecules suitable for use in various different application pathways.

The raw cellulose-containing feed material may be substantially homogeneous (e.g., pre- or post-consumer waste, scrap textile fiber and fabric, cotton-containing fabrics, biomass or pulped wood or biomass, etc.), or it may be at least somewhat heterogeneous (e.g., cellulose-containing materials from mixed sources and of mixed types). When post-consumer textile materials are used as feedstock, used clothing collection and sorting may be accomplished via clothing retailers, manufacturers, recyclers, and various other organizations, providing access to large volumes of used, cellulose-containing garments and scrap materials that would otherwise be discarded. Depending on the type and homogeneity of the cellulose-containing feedstock, optional sorting and removal of non-cellulosic components may be carried out prior to pretreatment of the cellulose-containing feedstock.

When reclaimed garments and textiles are used as cellulose-containing feed material, initial sorting of reclaimed garments and textiles according to fiber content may be advantageous prior to feedstock pretreatment and dissolving. In some embodiments, for example, reclaimed material (e.g., garments and textiles) may be sorted by cellulosic content—e.g., reclaimed materials may be separated into groups having different cellulosic contents, such as >90% or >80% or >70% or >50%, or other cellulosic contents, and less than 50% cellulosic content. Reclaimed fabric material having other fiber contents and compositions may also be sorted and separated, and reclaimed material may also be sorted by composition, such as separating cotton-wool blends, cotton-polyester blends, cotton-elastane blends, cotton-spandex blends, and the like. Separation of non-cellulosic-containing materials such as buttons, zippers, and the like may take place at the time of or following sorting and process pretreatment. Likewise, mechanical sizing or comminution, such as shredding, pulling, grinding, cutting, tearing, and the like may take place prior to or following sorting and process pretreatment.

Cellulosic feedstocks such as reclaimed garments and textiles typically incorporate a variety of dyes and/or chemical finishes and may be contaminated with other materials, such as dirt, grease, and the like. Other types of cellulosic feedstocks, such as biomass, postconsumer waste, and the like, also contain contaminants that are desirably removed prior to a pulping stage. Raw cellulose-containing feedstock (optionally treated to remove non-cellulose-containing materials, and optionally sized) is typically processed in one or more pre-treatment stage(s) to remove dyes, finishes, contaminants (oils, grease, etc.) and the like from the feedstock. Cellulosic feedstocks including textile materials may optionally be mechanically treated to provide smaller sized, or more uniformly sized, feedstock. The fabric feedstock may be sized if desired, such as by shredding, to provide a sized feedstock having a fragmented, high surface area for fiber pulping. Feedstock sizing is typically accomplished using mechanical cutting, shredding, or other mechanical size reduction techniques. Processing to remove

non-cellulosic components, such as buttons, zippers, fasteners, and the like may take place, if desired, prior to and/or following pretreatment.

Several different pre-treatment stages are described below, and various combinations of pretreatment stages may provide benefit, depending on the nature of the cellulosic feedstock. Depending on the properties of the raw textile feedstock, one or more of the pretreatments may be used, alone or in combination with other pretreatments. Several 10 (optional) pre-treatment stages are described below, and several advantageous pre-treatment combinations are also described. It will be appreciated that additional pre-treatments may be used in combination with the pre-treatments described, and that various specific combinations other than those specifically illustrated and described may be used.

FIG. 1 illustrates an overall process flow diagram for treating cellulose-containing materials to produce isolated cellulose polymers, identified in FIG. 1 as “Liquefied Cellulose,” suitable for use in a variety of downstream applications, such as fiber production (e.g., textiles, technical fibers and geo-textiles), production of other extrusion and/or constructional manufacturing methods (e.g., 3D printing media, membranes, injection molding media), use as a chemical feedstock for production of biofuels, lubricants 20 and other chemical manufacturing, and for use as food additives, in films, coating, fillers, membranes, packaging, construction materials, non-woven materials, and the like. FIG. 2 illustrates an overall process flow diagram for treating cellulose-containing materials to produce liquefied cellulose suitable for fiber extrusion and including additional 25 processing stages for production of regenerated cellulosic fiber. In some embodiments, fibers extruded from liquefied cellulose produced according to the overall process of FIG. 2 may be used as feed to produce carbonized and graphitized 30 materials. The cellulose-containing materials may undergo similar pretreatment and dissolution stages, as illustrated in FIGS. 1 and 2, while the isolated cellulose product may be used for different applications, as shown.

In general, cellulose-containing feed materials may 40 undergo optional feedstock preparation stages, such as feedstock sorting and/or removal of non-cellulosic components. The cellulose-containing feedstock then undergoes at least one pretreatment stage, followed by dissolution of the pretreated cellulose-containing feedstock and filtration to produce 45 isolated cellulose polymers. Several pretreatment stages are described below and are illustrated in the accompanying diagrams. Depending on the composition of the cellulose-containing feedstock and the attributes of the cellulosic product desired, one or more than one of the pretreatment stages may be used alone or in combination with other pretreatment stages. Specific combinations of pretreatments that may be useful in particular applications are 50 described in greater detail below with reference to FIGS. 3-7. Each of the pretreatment stages is described in more detail below.

#### High Temperature Aqueous Washing

In one embodiment, methods disclosed herein provide pretreatment of cellulose-containing feed materials using a high temperature aqueous washing process. This pretreatment 60 stage is particularly useful for pretreatment of cellulose-containing feed materials comprising recycled garments and may facilitate removal of contaminants such as soils, deodorants, lanolin, silicone and cationic softeners from the feedstock, as well as stripping various fabric treatments, such as optical brighteners, moisture wicking enhancers, and the like, from the feed material. Aqueous media maintained at a temperature above 100° C., optionally

above the boiling point of the aqueous media, generally above 120° C., often between 120° C. and 170° C., sometimes between 130° C. and 150° C., and up to 200° C., may be used. In some embodiments, the high temperature aqueous washing pretreatment stage is conducted in a closed vessel batch system with circulation or agitation or mixing of the hot aqueous media. Pressure conditions in a closed vessel system, as described, may range from about 100 kPa to about 2000 kPa, depending on the temperature of the aqueous media, with higher pressure conditions accompanying higher temperature media.

Aqueous media used in a high temperature pretreatment stage may comprise water alone, or it may comprise an aqueous solution having one or more additives. In some embodiments, the aqueous media may comprise water enriched with ozone. In some embodiments, the aqueous media may comprise water enriched with oxidative agents such as hydrogen peroxide or sodium perborate. In additional embodiments, surfactants (e.g., Sodium stearate, Fatty Alcohols, 4-(5-Dodecyl) benzenesulfonate, Alcohol ethoxylates and the like) and/or various hydroxide compositions (e.g., Ca, Mg, Na, K, and Li hydroxides), may be mixed and circulated with the aqueous media in a high temperature aqueous pretreatment stage and may act as wetting agents.

In some embodiments, the high temperature aqueous washing stage incorporates an aqueous solution comprising NaOH at a concentration of from about 1% to about 15%, at a pH in excess of about 11, and in some embodiments in excess of about 12. Residence times are sufficient to substantially remove impurities from the cellulose-containing feedstock.

The aqueous wash solution may be evacuated following a suitable residence time. In some embodiments, multiple aqueous washing stages may be implemented, using the same or different aqueous solutions, all at high temperature and pressure conditions. Optional rinsing of the solids with an aqueous solution may be implemented following evacuation of the wash solution. Rinsing may take place at ambient temperatures and pressures, with optional agitation and mixing, and the rinse solution is removed following a suitable residence time. Cellulose-containing treated solids may undergo one or more additional pretreatment stage(s) or may be further processed in a pulping and/or dissolution stage.

#### Supercritical CO<sub>2</sub> Washing

In some embodiments, a water-less and/or "non-toxic" pretreatment may be used to remove contaminants such as dyes, finishes, surface impurities and other contaminants from cellulose-containing feed materials, and particularly from feed materials comprising recycled garments or textiles. In this treatment stage, cellulose-containing feed material may be introduced to a closed and pressurized chamber, where the feed material contacts supercritical carbon dioxide, alone or in combination with additional reagent(s). In some embodiments, the supercritical CO<sub>2</sub> may be enriched with ozone. In some embodiments, the supercritical CO<sub>2</sub> may be enriched with oxidative agents such as hydrogen peroxide or sodium perborate. In additional embodiments, surfactants (e.g., Sodium stearate, Fatty Alcohols, 4-(5-Dodecyl) benzenesulfonate, Alcohol ethoxylates and the like) may be mixed and circulated with the supercritical CO<sub>2</sub> in a pretreatment stage. Following a suitable residence time, supercritical carbon dioxide containing dissolved contaminants is withdrawn to a separator, where the carbon dioxide may be decompressed and returned to a gaseous state, while the contaminants may be collected and removed. The gaseous carbon dioxide may be recycled in a closed

loop process and re-used for additional pretreatment cycles. Cellulose-containing treated solids may undergo one or more additional pretreatment stage(s) or may be further processed in a dissolution stage.

#### 5 Amorphous Phase Aqueous Treatment

In some embodiments, cellulose-containing feedstock (and/or cellulose-containing treated solids) is treated, prior to dissolution, with a high temperature (>320° C.), high pressure (>2.5 Mps) aqueous treatment, in a closed and substantially rigid reaction vessel. This pretreatment stage promotes breakdown of the crystalline structure of cellulose and facilitates modification of cellulosic constituents to an amorphous, non- or less-crystalline structure that is more amenable to pulping and/or dissolution.

#### 15 Treatment with Oxidative and/or Reducing Agent(s)

In some embodiments, a pretreatment stage involves exposing the cellulose-containing feed material (and/or cellulose-containing treated solids) to a "bleaching" agent, such as an oxidative or reducing agent, typically in an aqueous solution, at an oxidative/reducing agent concentration and for a residence time sufficient to remove materials such as dyes, finishes, and other contaminants from the cellulosic feedstock. Suitable oxidative and/or reducing agents include, for example, peroxide compositions (e.g., H<sub>2</sub>O<sub>2</sub>, 20 Na<sub>2</sub>O<sub>2</sub>) and perborate (e.g., NaBO<sub>3</sub>) compositions. Additional oxidative and/or reducing agents that may be used in pretreatment stages as described herein include one or more of the following compositions: per carbonate compositions; sodium carbonate; per acetic acid compositions; potassium 25 permanganate; persulfate compositions; ozone; sodium chloride; calcium oxychloride, sodium hypochlorite; calcium hypochlorite; lithium hypochlorite; cloramine; isocynual trichloride; Sulphur dioxide; sodium hydrosulfite; sulphoxylates; acidic sodium sulphite; sodium bosulphite; 30 sodium meta bisulphite; TAED (tetra-acetyl-ethylene-diamine); and sodium hydrosulfite.

In some embodiments, bleaching agent treatment may involve treatment in an aqueous solution of calcium hypochloride (bleach powder) or sodium hypochlorite (NaOCl) 40 in combination with sodium carbonate (soda ash) at a pH in excess of 8 and, in some embodiments, at a pH in excess of 9. Agitation or mixing of the materials in the bleaching agent pretreatment stage may be provided, and treatment with an oxidative and/or reducing agent may take place in a closed 45 reaction vessel.

The bleaching agent solution may be evacuated following a suitable residence time and optional rinsing of the solids with an aqueous solution may be implemented. Aqueous rinsing may take place at ambient temperatures, with the 50 rinse solution removed following a suitable residence time. The bleaching agent may be neutralized, following this treatment, by introduction of a weak acid such as hydrogen peroxide. In some embodiments, multiple bleaching agent treatment cycles may be implemented using different oxidative 55 or reducing reagents to treat the solids at different concentrations, pH conditions, temperature and/or residence times, as appropriate. Recycling and regeneration of the oxidative or reducing agent(s) may be incorporated in the process, as is known in the art. Introduction of other weak acids may be effective to reduce the pH of the treated, cellulose-containing solids, if desired, following optional rinsing steps.

#### Pretreatment with Organic Solvent(s)

In some embodiments, methods disclosed herein provide 60 pretreatment of cellulose-containing feed materials (and/or cellulose-containing treated solids) by exposure to aqueous media containing one or more organic solvents. Suitable

organic solvents may be selected from the group consisting of: acetic acid; acetone; acetonitrile; benzene; 1-butanol; 2-butanol; 2-butanone; t-butyl alcohol; carbon tetrachloride; chlorobenzene; chloroform; cyclohexane, 1,2-dichloroethane; diethylene glycol; diethyl ether; diglyme (diethylene glycol dimethyl ether); 1,2-dimethoxy-ethane (glyme, DME); dimethyl formamide (DMF); dimethyl sulfoxide (DMSO); 1,4-dioxane; ethanol, ethyl acetate; ethylene glycol; glycerin; heptane; hexamethylphosphoramide (HMPA); hexamethylphosphorous tramide (HMPT); hexane; methanol; methyl t-butyl ether (MTBE); methylene chloride; nitromethane; pentane; 1-propanol; 2-propanol; pyridine; tetrahydrofuran (THF); toluene; triethyl amine; o-xylene; and m-xylene. The aqueous media containing organic solvent(s) is generally maintained at a basic pH, generally at a pH in excess of 9, and often at a pH of 10 or above. Treatment with organic solvents may be achieved using high temperature or cooler aqueous media.

#### Enzymatic Treatment

In some embodiments, methods disclosed herein may optionally employ enzymatic treatment to shorten cellulose molecules, increase cellulose solubility and/or reduce reaction times in subsequent treatment stages. Suitable enzymes may include endoglucanases (e.g., Cel 5A, Cel 7B, Cel 12A, Cel 45, Cel 61A); Cellobiohydrolases (e.g., Cel 6A, Cel 7A); LPMO/GH61; cellulases; and the like. In general, temperatures of from about 30° to 90° C., pH between about 4 to about 9 and dwell times of from about 20 min to 48 hours may be suitable for enzymatic treatment.

Enzymatic treatment(s) involving xylanases, alkaline pectinases, lipases, and/or esterases may also be used for feedstock pretreatment prior to pulping. In yet additional embodiments, feedstock may be treated using enzymatic cultures containing biological organisms (fungi, bacteria, etc.) that secrete cellulolytic enzymes (e.g., cellulases). Enzyme cultures such as *Trichoderma Reesei*, *Trichoderma viride*, *Penicillium janthinellum*, *Halorhabdusutahensis*, *A Niger*, *Humicola*, and mixtures of such enzyme-producing cultures, are suitable. Mechanical treatments such as pulv-erization and/or emulsification treatment(s) may be implemented following enzymatic treatment.

#### Treatment with Swelling Agents

For some applications (for example, those in which natural or light-colored or undyed regenerated fiber is desired as an end-product), an optional cellulose activation treatment using a swelling agent, such as an ionic liquid, may be employed prior to a cellulose dissolving stage to enhance the absorption penetration and synergistically increase the efficacy of a subsequent dissolving phase. Treatment with a swelling agent (e.g., an ionic liquid) may be preceded by or implemented in combination with one or more other pre-treatment stage(s). All of the swelling agents listed below may be used alone or in combination, and different swelling agents and swelling agent combinations may be desirable for different feedstock compositions and constituents. In some embodiments, swelling agents may be used alone, or in combination, at specific temperatures, concentrations and conditions to directly dissolve the cellulose without requiring a downstream dissolving stage. The efficacy of treatment with swelling agents such as ionic liquids, and the ability to use a swelling agent (e.g., ionic liquid) as a direct cellulose dissolving reagent may depend on various factors including, for example, on the degree of polymerization of the cellulose being dissolved.

Suitable ionic liquids may comprise hydroxides, such as Ca, Mg, Na, K, and/or Li hydroxides. Swelling agents suitable for use as reagents in a pretreatment stage may

alternatively or additionally comprise one or more of the following reagents: [AMIM]Cl 1-Allyl-3-methylimidazolium chloride; [BzPy]Cl Benzylpyridinium chloride; [BMIM]Ace 1-Butyl-3-methylimidazolium acesulphamate; [BMIM]DBP 1-Butyl-3-methylimidazolium dibutylphosphate; [BMIM]Cl 1-Butyl-3-methylimidazolium chloride; [BMIM]PF6 1-Butyl-3-methylimidazolium hexafluorophosphate; [BMIM]BF4 1-Butyl-3-methylimidazolium tetrafluoroborate; [BMPy]Cl 1-Butyl-3-methylpyridinium chloride; [DBNH]AcO 1,8-Diazabicyclo[5.4.0]undec-7-enium acetate; [DBNH]EtCOO 1,8-Diazabicyclo[5.4.0]undec-7-enium propionate; [DMIM]DEP 1,3-Dimethylimidazolium diethylphosphate; [DMIM]DMP 1,3-Dimethylimidazolium dimethylphosphate; [EMBy]DEP 1-Ethyl-3-methylbutylpyridinium diethylphosphate; [EMIM]AcO 1-Ethyl-3-methylimidazolium acetate; [EMIM]Br 1-Ethyl-3-methylimidazolium bromide; [EMIM]DBP 1-Ethyl-3-methylimidazolium dibutylphosphate; [EMIM]DEP 1-Ethyl-3-methylimidazolium diethylphosphate; [EMIM]DMP 1-Ethyl-3-methylimidazolium dimethylphosphate; [EMIM]MeSO4 1-Ethyl-3-methylimidazolium methanesulphonate; [HPy]Cl 1-Hexylpyridinium chloride; [E(OH)MIM]AcO 1-Hydroxyethyl-3-methylimidazolium acetate; [DBNMc]DMP 1-Methyl-1,8-diazabicyclo[5.4.0]undec-7-enium dimethylphosphate; [P4444]OH Tetra-butylphosphonium hydroxide; [TMGH]AcO 1,1,3,3-Tetramethylguanidinium acetate; [TMGH]n-PrCOO 1,1,3,3-Tetramethylguanidinium butyrate; [TMGH]COO 1,1,3,3-Tetramethylguanidinium formate; [TMGH]EtCOO 1,1,3,3-Tetramethylguanidinium propionate; [P8881]AcO Trioctylmethylphosphonium acetate; and HEMA Tris-(2-hydroxyethyl)methylammonium methylsulphate.

In one exemplary embodiment, cellulose-containing feed materials (and/or cellulose-containing treated solids) may be treated with an ionic solution such as an aqueous solution comprising Ca, Mg, Na, K, and/or Li hydroxides, optionally followed by exposure to a sodium hydrosulfite ( $Na_2S_2O_4$ ) reducing agent and/or a bleaching agent such as peroxide, perborate, persulfate, and sodium or calcium hypochlorite. Small amounts of Bromium (Br) may be used as a catalyst during this treatment. This treatment is generally carried out at a pH in excess of 9, and often at a pH of 10 or 10.5 or above. Treatment with swelling/dissolving agents such as ionic liquids may be achieved using high temperature or cooler aqueous wash media. In some embodiments, treatment with a swelling agent (e.g., an ionic liquid) is conducted at temperatures of 0° C. or lower, provided the aqueous solution or slurry is prevented from freezing, and provided the viscosity of the solution is maintained at an acceptable level. In some embodiments, and particularly when ionic liquids having an acetate group are used, the treatment may be carried out at an acidic pH, typically at a pH less than 6, and in some embodiments at a pH less than 5. In some embodiments, the proportion of cellulose-containing feed materials (and/or cellulose-containing treated solids) in the ionic solution is from about 2% to about 40%; in some embodiments, the proportion of cellulose-containing feed materials (and/or cellulose-containing treated solids) in the ionic solution is from about 5% to about 25%.

It will be appreciated that numerous (optional) pretreatment processes are described herein and are illustrated in FIGS. 1 and 2. Pretreatment of cellulose-containing feedstock material, as described, may implement any of these pretreatment processes, singly or in combination with one or more other pretreatment processes. In some embodiments, carrying out elevated temperature aqueous pretreatment in a closed vessel is preferred, alone or in combination with other

pretreatment stages, prior to pulping and dissolution of the cellulose polymers. In some embodiments, carrying out elevated temperature aqueous pretreatment with the use of ozone enrichment, oxidative agents and/or surfactants is preferred, alone or in combination with other pretreatment stages, prior to pulping. In some embodiments, treatment in ionic solution followed by exposure to a reducing and/or bleaching agent is preferred, preferably in combination with a washing step. In some embodiments, pretreatment involves elevated temperature aqueous pretreatment, followed by ionic pretreatment, followed by enzymatic pretreatment. In some embodiments, one or more of the pretreatment stages, or all pretreatment stages, are carried out a pH of at least about 9. In some embodiments, one or more of the pretreatment stages, of all of the pretreatment stages, are carried out at a pH of at least about 10.

Pretreatment preferably takes place in a closed vessel and, in batch treatment schemes, one or more pretreatment reagents may be introduced to and withdrawn from a closed vessel during various pretreatment stages, with or without intermediate rinsing or washing stages. In some embodiments, the vessel may be provided in the form of a rotating cylinder with a pressurized hull (housing) capable of withstanding pressures in the range of from 1000-5000 kPa, having inlet and outlet ports, pH and rpm control features, and having liquid agitation or circulation features. The inner reaction vessel surfaces may comprise anticorrosive metal(s) capable of withstanding concentrated acidic and alkali solutions. In some processes, both pretreatment and dissolution may take place in the same vessel.

Specific pretreatment combinations are described below with reference to the schematic flow diagrams shown in FIGS. 3-7. Each of these flow diagrams describes different feedstock pretreatment combinations, followed by molecular isolation and separation of cellulose polymers in a dissolution stage. Cellulose polymers may be separated from the dissolution solution, such as by filtration, and regenerated cellulosic fibers may be extruded, such as in connection with a precipitation bath (e.g., an acid bath). Extruded fibers may be designed and parameters changed, depending on the type, character and physical attributes of the cellulosic fibers desired. Drying and winding produces regenerated cellulosic fibers.

FIG. 3 illustrates treatment of cellulose-containing materials (with optional sorting and removal of non-cellulosic components) using a high temperature aqueous wash or supercritical carbon dioxide pretreatment stage in combination with ozone enrichment and/or oxidative agent(s) and/or surfactant(s). Following evacuation of the hot aqueous or supercritical CO<sub>2</sub> media used for washing, and optional rinsing of the cellulosic solids, the cellulosic solids may optionally be treated with swelling agents (as described above), and/or with organic solvents (again, as described above). These treatment stages may be done at elevated temperatures or in cooler-aqueous media.

FIG. 4 illustrates treatment of cellulose-containing materials (with optional sorting and removal of non-cellulosic components) using a high temperature aqueous wash or supercritical carbon dioxide pretreatment stage in combination with oxidative agent(s) and/or surfactant(s). Following evacuation of the hot aqueous or supercritical CO<sub>2</sub> media used for the washing stage, and following optional rinsing of the cellulosic solids, the cellulosic solids may optionally undergo enzymatic treatment as described above. The cellulosic solids may subsequently be exposed to swelling agents such as ionic liquids (e.g., NaOH) prior to a dissolution stage.

FIG. 5 illustrates treatment of cellulose-containing materials (with optional sorting and removal of non-cellulosic components) using a high temperature aqueous wash or supercritical carbon dioxide pretreatment stage in combination with oxidative agent(s) and/or surfactant(s). Following evacuation of the hot aqueous or supercritical CO<sub>2</sub> media used for the washing stage, and following optional rinsing of the cellulosic solids, the cellulosic solids may optionally be exposed to swelling agents such as ionic liquids (e.g., NaOH), followed by enzymatic treatment as described above prior to a dissolution stage.

FIG. 6 illustrates treatment of cellulose-containing materials (with optional sorting and removal of non-cellulosic components) using a high temperature aqueous wash or supercritical carbon dioxide pretreatment stage in combination with optional ozone enrichment and/or oxidative agent(s) and/or surfactant(s). Following evacuation of the hot aqueous or supercritical CO<sub>2</sub> media used for the washing stage, and following optional rinsing of the cellulosic solids, the cellulosic solids may optionally be exposed to swelling agents such as ionic liquids (e.g., NaOH), followed by exposure to bleaching agents and/or reducing agents and/or an optional enzyme treatment, all as described above, prior to a dissolution stage.

FIG. 7 illustrates treatment of cellulose-containing materials (with optional sorting and removal of non-cellulosic components) using a high temperature aqueous wash or supercritical carbon dioxide pretreatment stage in combination with optional ozone enrichment and/or oxidative agent(s) and/or surfactant(s). Following evacuation of the hot aqueous or supercritical CO<sub>2</sub> media used for the washing stage, and following optional rinsing of the cellulosic solids, the cellulosic solids may optionally undergo a high-temperature, high-pressure aqueous treatment stage, as described above, to promote destruction of the cellulosic crystalline structure and favor conversion of cellulosic polymers to an amorphous phase. The cellulosic solids may be exposed to enzyme treatment, as described above, prior to a dissolution stage.

Treated cellulose-containing solids are subjected to a dissolving stage, in which the cellulose-containing solids are treated in a dissolving reagent to promote molecular separation of cellulose polymers and destruction of intermolecular hydrogen bonds and other non-covalent bonds, converting cellulose-containing solids to their constituent cellulose polymers. In some embodiments, the number of intermolecular hydrogen bonds present in the cellulose polymers is reduced by at least 20% in the fiber pulping stage; in some embodiments, the number of intermolecular hydrogen bonds present in the cellulose polymers is reduced by at least 50% in the fiber pulping stage; in yet other embodiments, the number of intermolecular hydrogen bonds present in the cellulose polymers is reduced by at least 70% in the fiber dissolving stage. The viscosity of dissolved cellulose, following the dissolution treatment, is generally from about 0.2 to as high as 900 cP, often from about 0.5 to about 50 cP.

A variety of cellulose dissolving techniques and cellulose dissolving chemistries are available, and one or more of the pretreatment stages described above may be used with a variety of known cellulose dissolving reagents, including those described in PCT Int'l Patent Publication WO 2013/124265 A1, the disclosure of which is incorporated herein by reference in its entirety.

In some embodiments, copper-containing reagents are preferred for use as cellulose dissolving reagents. In one embodiment, for example, Schwiezer's Reagent—(the

chemical complex tetraaminecopper (II) hydroxide— $[\text{Cu}(\text{NH}_3)_4(\text{H}_2\text{O})_2]^{2+}$  or tetraamminediaquacopper dihydroxide,  $[\text{Cu}(\text{NH}_3)_4(\text{H}_2\text{O})_2](\text{OH})_2$  is a preferred cellulose dissolving reagent to isolate and promote molecular separation of cellulose polymers. Schweizer's reagent may be prepared by precipitating copper(II) hydroxide from an aqueous solution of copper sulfate using sodium hydroxide or ammonia, then dissolving the precipitate in a solution of ammonia. In some embodiments, a combination of caustic soda, ammonium and cupramonium sulfate may be formulated to provide Schweizer's Reagent.

Solutions comprising copper(II) hydroxide and ammonia may be introduced and used in the cellulose dissolving stage to form Schweizer's Reagent according to the following reaction:  $\text{Cu}(\text{OH})_2 + 4 \text{NH}_3 + 2 \text{H}_2\text{O} \rightarrow [\text{Cu}(\text{NH}_3)_4(\text{H}_2\text{O})_2]^{2+} + 2 \text{OH}^-$ . In this scheme, the copper hydroxide reagent may be manufactured from recycled copper recovered, for example, from electronics and computer component waste materials. Copper hydroxide is readily made from metallic copper by the electrolysis of water using copper anodes. Ammonia may be manufactured by an innovative use of the Haber-Bosch process ( $3 \text{H}_2 + \text{N}_2 \rightarrow 2 \text{NH}_3$ ), capturing hydrogen from organic wastes and combining it with atmospheric nitrogen. This method may produce ammonia at low cost and eliminate greenhouse gas emissions from organic waste feedstock. Using these reagent resources and methods for generating Schweizer's Reagent, all or substantially all of the materials used in the cellulose dissolving process described herein (including the cellulose-containing feedstock) may be sourced as waste products, resulting in minimal or no use of nonrenewable resources.

Other cellulose-dissolving agents may also be used in the cellulose dissolving stage, such as iron-containing and zinc-containing reagents. In one embodiment, iron tartrate complex solvents (e.g., FeTNa) may be used as cellulose dissolving reagents. FeTNa solutions may be prepared according to the procedure published by Seger et al. (B. Seger, et al., *Carbohydrate Polymers* 31 (1996) 105.) FeTNa solutions are prepared and stored while protecting them from light. The FeTNa complex may be prepared, for example, by dissolving sodium tartrate dehydrate (Alfa Assar, Cat. #16187) in deionized water, stirring and optionally heating. When the sodium tartrate dissolved, iron nitrate nonahydrate (Alfa Aesar, Cat. #12226) is added to the solution with continuous stirring. The solution is then cooled to 10-15° C. to prevent precipitation of the iron complex. 12 M sodium hydroxide solution is slowly added to the tartrate-ferric acid under controlled conditions to prevent the temperature from rising over 20° C. The solution color shifts from reddish-brown to yellowish-green, signifying the formation of the FeTNa complex. After this transition, the remaining sodium hydroxide may be added-without regard to temperature. Sodium tartrate is added at the end to ensure long-term stability of the solution.

Cellulose dissolving conditions using an FeTNa dissolving reagent are generally basic and may be carried out at pH above 12, or above 13, or at a pH of about 14 in a closed reaction vessel. Reactions carried out using FeTNa dissolving reagent at a pH of 14 in a closed reaction vessel kept at 4° C. successfully dissolved cotton feedstock. Carrying out the cellulose dissolving reaction in an inert atmosphere is generally preferred, and circulating an inert gas such as argon through the cellulose dissolving solution prior to and during addition of pretreated feedstock may improve dissolution rates and/or yields.

In another embodiment, zinc-containing reagents such as Zincoxen solutions may be used as cellulose dissolving

reagents. The active ingredients of the Zincoxen solution are zinc oxide (ZnO) and EDA. Zincoxen solutions may be prepared according to the procedures published by Shenouda and Happey (S. G. Shenouda and F. Happey, *European Polymer Journal* 12 (1975) 289) or Saxena, et al. (V. P. Saxena, et al., *Journal of Applied Polymer Science* 7 (1963) 181). Ethylenediamene-water solutions are chilled to 0° C. followed by stirring in zinc oxide powder. Continuous stirring for 72 hours while maintaining the temperature at 0° C. produces a suitable Zincoxen solution. Cellulose dissolving conditions using a Zincoxen cellulose dissolving reagent are generally basic and may be carried out at pH above 12, or above 13, or at a pH of about 14 in a closed reaction vessel.

In general, residence times of up to 4-48 hours in the cellulose dissolving stage are suitable to dissolve and promote molecular separation of cellulose molecules present in the treated cellulose-containing feedstock. In some embodiments, the cellulose dissolving stage takes place in a closed chamber and an inert gas, such as nitrogen or argon, is introduced in the airspace to inhibit or prevent oxidation of cellulose dissolving solution constituents. Oxygen-containing gases may be substantially evacuated from the cellulose dissolving stage. In some embodiments, agitation and/or mixing of the cellulose dissolving mixture may be provided; in some embodiments, an inert gas, such as nitrogen or argon, may be bubbled through the cellulose dissolving mixture prior to and/or during cellulose dissolution.

FIG. 9 illustrates a cellulose dissolution stage in which pretreated cellulosic material is treated with a dissolving solvent, wherein the solvent is selected from the group consisting of: ionic liquids; metal alkali system complexes; organic solvents; and other solvents, such as sulfuric acid, xanthogenation; or combinations thereof. FIG. 10 cites exemplary ionic liquids, alkaline metal system complexes, organic solvents, alkaline xanthogenation reagents, and other solvents. Any of these solvents may be used, alone or in combination, to break hydrogen bonds between cellulose molecules and produce isolated cellulose molecules in the cellulose dissolving stage. Solvents that may be used in the cellulose dissolving stage include: Alkaline Metal System Complexes such as  $[\text{Cu}(\text{NH}_3)_4(\text{OH}_2)_2$  (cuoxam),  $[\text{CuH}_2\text{NCH}_2\text{CH}_2\text{NH}_2]_2(\text{OH})_2$  (cuen), Cupriethylenediamine (CED),  $[\text{Ni}(\text{NH}_3)_6(\text{OH})_2]$ ,  $[\text{Cd}(\text{H}_2\text{NCH}_2\text{CH}_3\text{NH}_2)_3(\text{OH})_2]$  (cadoxen),  $[\text{Zn}(\text{H}_2\text{NCH}_2\text{CH}_2\text{NH}_2)_3(\text{OH})_2]$ ,  $[\text{Fe}_3(\text{tartrate acid})_3\text{NaOH}]$  (EWNN) and LiOH; organic solvents such as  $[\text{Cl}_3\text{CHO}/\text{DMF}, (\text{CH}_2\text{O})_x/\text{DMSO}, \text{N}_2\text{O}_4/\text{DMSO}, \text{Li}/\text{DMAc}(\text{N,N-dimethylacetamide}), \text{LiCl}/\text{DMI}(\text{N,N-dimethylimidazolidinone}), \text{SO}_2/\text{amine}/\text{DMSO}, \text{CH}_3\text{NH}_2/\text{DMSO}, \text{CF}_3\text{COOH}$ , alkaline Xanthogenation compositions such as  $[\text{CS}_2/\text{NaOH}$ , other solvents such as  $[\text{ZnCl}_2 (<64\%), \text{Ca}(\text{SCN})_3 (>50\%), \text{Bu}(4\text{N}^+\text{F}-3\text{H}_2\text{O})/\text{DMSO}, \text{NH}_4\text{SCN}/\text{NH}_3/\text{water}, \text{CO}(\text{NH}_2)_2$  (urea),  $\text{H}_2\text{SO}_4 (>52\%)$  (sulfuric acid), ionic liquids such as  $[\text{NMNO}]^+\text{N-methylmorpholine-N-oxide}; [\text{AMIM}]^+\text{Cl}^-$  1-Allyl-3-methylimidazolium chloride;  $[\text{BzPy}]^+\text{Cl}^-$  Benzylpyridinium chloride;  $[\text{BMIM}]^+\text{Ac}^-$  1-Butyl-3-methylimidazolium acesulphamate;  $[\text{BMIM}]^+\text{DBP}^-$  1-Butyl-3-methylimidazolium dibutylphosphate;  $[\text{BMIM}]^+\text{Cl}^-$  1-Butyl-3-methylimidazolium chloride;  $[\text{BMIM}]^+\text{PF}_6^-$  1-Butyl-3-methylimidazolium hexafluorophosphate;  $[\text{BMIM}]^+\text{BF}_4^-$  1-Butyl-3-methylimidazolium tetrafluoroborate;  $[\text{BMPy}]^+\text{Cl}^-$  1-Butyl-3-methylpyridinium chloride;  $[\text{DBNH}]^+\text{AcO}^-$  1,8-Diazabicyclo[5.4.0]undec-7-enium acetate;  $[\text{DBNH}]^+\text{EtCOO}^-$  1,8-Diazabicyclo[5.4.0]undec-7-enium propionate;  $[\text{DMIM}]^+\text{DEP}^-$  1,3-Dimethylimidazolium diethylphosphate;  $[\text{DMIM}]^+\text{DMP}^-$  1,3-Dimethylimidazolium dimethylphosphate;  $[\text{EMBy}]^+\text{DEP}^-$

1-Ethyl-3-methylbutylpyridinium diethylphosphate; [EMIM]AcO 1-Ethyl-3-methylimidazolium acetate; [EMIM]Br 1-Ethyl-3-methylimidazolium bromide; [EMIM]DBP 1-Ethyl-3-methylimidazolium dibutylphosphate; [EMIM]DEP 1-Ethyl-3-methylimidazolium diethylphosphate; [EMIM]DMP 1-Ethyl-3-methylimidazolium dimethylphosphate; [EMIM]MeSO<sub>4</sub> 1-Ethyl-3-methylimidazolium methanesulphonate; [HPy]Cl 1-Hexylpyridinium chloride; [E(OH)MIM]AcO 1-Hydroxyethyl-3-methylimidazolium acetate; [DBNMc]DMP 1-Methyl-1,8-diazabicyclo[5.4.0]undec-7-enium dimethylphosphate; [P4444]OH Tetraethylphosphonium hydroxide; [TMGH]AcO 1,1,3,3-Tetramethylguanidinium acetate; [TMGH]n-PrCOO 1,1,3,3-Tetramethylguanidinium butyrate; [TMGH]COO 1,1,3,3-Tetramethylguanidinium formate; [TMGH]EtCOO 1,1,3,3-Tetramethylguanidinium propionate; [P8881]AcO Trioctylmethylphosphonium acetate; HEMA Tris-(2-hydroxyethyl)methylammonium methylsulphate; and [DBN-Me]DMP 1-Methyl-1,8-diazabicyclo[5.4.0]undec-7-enium dimethylphosphate and Ca, Mg, Na, K, and/or Li hydroxides. These compounds may be used alone or in various combinations as cellulose dissolving agents.

In some embodiments, one or more ionic liquids, such as 1-Ethyl-3-methylimidazolium [EMIM] compositions, may be used as cellulose dissolving agents. 1-Ethyl-3-methylimidazolium [EMIM] compositions comprising at least one polar group such as EMIM acetate, bromide, dibutylphosphate, diethylphosphate, dimethylphosphate, or methanesulphonate compounds are suitable for many applications. Combinations of ionic liquids may be used. In some embodiments, Ca, Mg, Na, K, and/or U hydroxides may be used in combination with any of the other cellulose dissolving solvents disclosed in the cellulose dissolving phase. The use of Ca, Mg, Na, K, and/or Li hydroxides in an amount of from about 1% to about 10% by volume in combination with any of the other cellulose dissolving solvents may enhance the cellulose dissolution process.

1-Ethyl-3-methylimidazolium acetate ([EMIM] AcO), is used in some embodiments as a cellulose dissolving agent for cellulosic feedstock such as cotton, cotton/poly blends and other post-consumer cellulosic waste feedstocks. EMIM AcO may be used in a nearly pure form (at least 70% pure in some embodiments; at least 80% pure in some embodiments; at least 90% pure in some embodiments; and about 95% to 98% pure in some embodiments). Pre-treated feedstock may be dried to a moisture content of less than about 25% in some embodiments, less than about 15% in some embodiments, less than about 10% in some embodiments, and less than about 5% in some embodiments, by heat treatment (e.g., feedstock treatment at temperatures of about 100° C. for a time sufficient to reduce the aqueous content of the feedstock to less than 25% or less than 15% or less than 10% or 5%). Treatment with an EMIM AcO ionic liquid cellulose dissolving agent generally takes place at a temperature of at least about 60° C. and up to about 120° C., and may take place at a temperature of about 85° C. to about 95° C. Feedstock loading of up to about 20% cellulosic material is generally suitable, with reaction times of from about 30 min to about 6 hours, depending on the feedstock concentration, the ionic liquid concentration, and the reaction temperature. Following dissolution of the cellulosic material, extrusion may be carried out with an air gap in an aqueous solution, such as water. The water temperature is preferably from about 5° and 95° C.

Treatment with a dissolving solvent may be accompanied by one or more of the following: introduction of an inert gas, such as nitrogen or argon (or another noble gas); introduc-

tion of mechanical and/or electrical energy; introduction of one or more conditional agents, such as glycerine; and filtration and scraping. Filtration and extrusion may then be carried out using the isolated cellulose molecules to produce cellulose for use in various applications, including in the manufacture of regenerated cellulosic fiber.

The cellulose molecules are substantially isolated and may be fully or partially dissolved to form substantially linear cellulose chains in the cellulose dissolution stage, 10 depending on the cellulose dissolving reagent used and the residence time. The cellulose dissolving solution is filtered, following a suitable residence time, to remove non-cellulosic constituents with the solution and isolate substantially purified cellulose polymers, which are typically suspended in a viscous media. Filtration may involve multiple stages, 15 including an optional centrifugation stage and one or more size exclusion filtration stages. A final filtration stage using pore sizes of 1 micron or less may be employed. The isolated, substantially purified cellulose polymers may be 20 used in a wide range of downstream applications (See, e.g., FIG. 1) and, in particular applications, are used in fiber production applications to produce regenerated cellulosic fiber (See, e.g., FIGS. 2-7).

In some embodiments, one or more high carbon content 25 compositions such as liquefied lignin(s), acrylic(s), pitch, and the like may be added to the cellulosic material during or following the cellulose dissolving stage and prior to extrusion to increase the carbon content of the dissolved cellulose, producing enhanced-carbon-content cellulosic 30 fibers, and to increase the fiber carbon content and yield. In some embodiments, liquefied lignin(s) may be added to the dissolved cellulosic material prior to extrusion in an amount of from about 2% to 20% of the pulp concentration to enhance the carbon content of cellulosic fibers produced. 35 Enhanced-carbon-content regenerated cellulosic fibers are particularly suitable for use as feedstock for carbonization processes.

The conditions of the cellulose dissolving stage and the 40 composition of the fabric feedstock are important factors in determining whether a cotton-like fiber or rayon is produced from the dissolved cellulosic materials in subsequent processing. Full dissolution of the cellulosic fibers is generally 45 desirable for the production of rayon-like fibers, cotton-like fibers and other regenerated cellulosic fibers. Suitable solvent concentrations, reagent to feedstock ratios, residence times, and the like, may be determined using routine experimentation. While Schwiezer's Reagent, iron- and zinc-containing cellulose dissolving reagents and ionic liquid 50 reagents described above are suitable cellulose dissolving solvents for many applications, it will be appreciated that other cellulose dissolving reagents may be available, or may be developed, and would be suitable for use in the processes described herein.

In some embodiments, energy is introduced to the dissolving solution during and/or following a desired degree of 55 dissolution. When the cellulose dissolving stage is carried out in a closed reaction chamber, mechanical and/or electrical energy, such as radio frequency energy, may be introduced during or following dissolution to enhance separation of different components and promote sedimentation of heavier components. If the cellulose-containing feedstock was not pretreated to remove non-cellulosic components, suitable filtration, screening and/or size exclusion treatment 60 may be performed, during or following cellulose dissolving, to remove non-organic materials (e.g., buttons, fasteners, zippers, etc.), as well as impurities and non-cellulosic materials from the dissolved fiber solution. Suitable filtration,

screening and/or size exclusion treatments will depend on the types and level of contaminants remaining in the dissolved fiber solution. Filtration may involve scraping the top and/or bottom of the reaction vessel to remove floating and/or sinking debris; simple size exclusion filtration; and/or gravitation separation or centrifugation to separate solids from the dissolved cellulosic materials. In some embodiments, a cascade of progressively smaller pore size filtration stages may follow preliminary separation by gravitation or centrifugation. Separated by-products may be isolated and purified (if appropriate) for re-sale or distribution to secondary markets.

In some embodiments, the cellulose dissolving solution may be optionally treated with glycerin or glycerol or another agent to impart softness to the texture of the fiber. **Fiber Extrusion**

After cellulose dissolution, isolated cellulose molecules may be extruded to form regenerated fibers and textile materials. The isolated cellulose molecules are generally filtered or otherwise separated, and may be acidified and processed in a wet extrusion stage to precipitate cellulose fibers and produce cotton fibers, rayon fibers, or a mixture of cotton and rayon fibers. Various acids may be used in this precipitation stage, such as sulfuric, citric or lactic acids. In one embodiment, a sulfuric acid bath is used in combination with a wet extrusion process, wherein the viscous cellulose polymer solution is pumped through a spinneret, and the cellulose is precipitated to form fibers as it contacts the acid bath. In some embodiments, depending on the dissolving agent as mentioned above, the extrusion may take place in warm aqueous solution (e.g., water) having a temperature of from about 5° and 95° C.

The extrusion process and/or system may be modified and adjusted to produce fibers having different lengths, diameters, cross-sectional configurations, durability, softness, moisture wicking properties, and the like. In this process, the newly formed fibers may be stretched and/or blown to produce desired configurations, washed, dried, and cut to the desired length. In some embodiments, dissolved cellulosic materials may be extruded through fine spinnerets that produce spun fibers having a diameter of about 50 microns, and the spun fibers may be additionally drawn to reduce the fiber diameter. Fibers having a diameter of less than 10 microns and having high strength have been generated using methods described herein, extruding from a precipitation bath having a solids content of from about 8% to 12% solids, followed by drawing to reduce the fiber diameter.

In some embodiments, "composite" fibers comprising two or more different compositions may be co-extruded using a twin extrusion methodology. In one exemplary method, dissolved cellulose generated using waste fabric feedstock, as described herein, is co-extruded with another dissolved carbon-based material, producing a composite fiber having distinct components (e.g., a regenerated cellulosic fiber component and another carbon-based fiber component). In some embodiments, the two or more distinct dissolved materials may be extruded in a sheath/core arrangement, with one dissolved carbon-containing composition extruded as a core fiber and a second dissolved carbon-containing composition extruded as a sheath that fully or partially covers the core fiber. In some embodiments, the two or more distinct carbon-containing compositions may be extruded in a side-by-side component arrangement, with one carbon-containing composition extruded to form a partial fiber cross-section and another composition extruded to form another partial fiber cross-section, the two partial fiber cross-sectional components forming a composite fiber. It

will be appreciated that composite fibers having different configurations, different compositions, and the like may be generated. Composite fibers composed of two or more different carbon-containing compositions may provide beneficial fiber properties and may confer beneficial environmental attributes.

Closed vat, continuous fiber extrusion techniques may be used. Closed vat systems allow recovery and/or recycling of any produced gases and by-products. Using fiber extrusion techniques is highly advantageous when applied to the regeneration of cellulosic materials to produce cotton and/or rayon fibers, since it allows a high degree of custom design and engineering of cellulosic fibers to achieve targeted comfort and performance characteristics (e.g., fiber length, diameter, cross-sectional shape, durability, softness, moisture wicking, etc.). Naturally grown fibers cannot be produced in desired or specified fiber lengths, diameters, cross-sectional profiles, or the like and cellulosic fibers regenerated using this process may therefore have different, and superior, properties compared to the natural fibers present in the initial recycled fabric feedstock.

In some embodiments, fiber extrusion may produce fibers having a denier of from about 0.1 to 70 or more. In some embodiments, fiber extrusion may involve extruding multi-filaments having from about 20 to 300 single monofilaments, each having a denier of from about 0.1 to about 2. Extruding fine denier filaments produces woven fabric that feels softer to the touch and is desired in many embodiments. In some embodiments, fiber extrusion may additionally involve adding a false twist to the extruded filaments and texturizing them to resemble spun yarn. These treatments may obviate the necessity of using opening and spinning processes to produce yarn from the extruded fibers. Further handling of the fibers may involve cutting the continuous fiber to specific uniform lengths (stapling), missing, opening, carding, drawing, rowing, spinning, etc.

Following fiber extrusion and spinning to form yarns, fabrics, textiles and the like, waterless dyeing techniques may be used to further reduce the environmental impact of the overall process. Waterless dyeing technologies are available and typically use supercritical carbon dioxide as a solvent and carrier for dyestuff. In some embodiments, color treatment of regenerated fibers may involve determining the absorbency of the regenerated fiber and determining the color properties of fibers using spectrophotometric techniques. Color signatures and dye formulations may then be customized according to the specific properties of regenerated fibers to eliminate differences in coloration that may result from different batch qualities. In some embodiments, regenerated fibers or yarns may be surface treated (e.g., using a bleaching composition) and then dyed or overprinted using, for example, reactive, direct, pigment, sulfur and/or vat dye types and prints. Regenerated cellulosic fibers (e.g., cotton and/or rayon) produced as described above may be twisted into thread, dyed, bleached, woven into textiles and, ultimately, cut and sewn into garments.

In some applications, all fiber regeneration process steps, from garment reclamation to fiber extrusion, may be located at a common geographic site (or at nearby sites). For some purposes, it may be desirable to locate different stages of the process at different physical locations. It may be desirable, in some applications, for example, to locate garment reclamation sites in populous areas, while locating other processing facilities and, in particular, the wet extrusion facility, in locations proximate textile processing facilities—e.g. near textile mills and/or garment manufacturing facilities. In some applications, garment reclamation and initial process-

ing may take place at one location and cellulosic pulp may then be shipped or transported to a different location for wet extrusion and other downstream processing (e.g., dying, garment manufacturing, etc.)

In another aspect, dissolution of low-grade cotton fibers, harvested naturally or produced from a raw material fabric feedstock as described above, is provided. In this process, low grade natural cotton fibers (e.g., low staple length cotton fibers) may be dissolved as described herein, and then acidified and subjected to a wet extrusion process to produce newly formed fibers which may be stretched and/or blown to a desired diameter, cross-sectional profile or the like, washed, dried, and cut to a desired length. In this fashion, low grade (natural and/or recycled) cotton fibers may be regenerated and converted to newly formed, higher value fibers having more desirable properties than those of the original natural and/or recycled cotton fibers.

In another aspect, process feedstock may comprise blended textile input comprising both cotton and polyester. FIG. 8 shows a schematic flow diagram illustrating the processing of a blended textile input according to methods described herein. In this scenario, blended textile input is separated into cotton-heavy and polyester-heavy blends during or following one or more sorting and pretreatment step(s). The constituent cotton and polyester polymers in each of the separated stages are dissolved and isolated to produce "liquefied" cellulose (i.e., isolated cellulose molecules) from the cotton-heavy feedstock and "liquefied" polyester (i.e., isolated polyester molecules) from the polyester-heavy feedstock. These isolated cellulosic and polyester materials may be extruded into regenerated fibers, as desired, or used for other downstream applications. The undissolved, non-cellulosic constituents remaining after dissolution of the cotton-heavy blend feedstock may be treated for dissolution of polyester to produce liquefied polyester. Likewise, the undissolved, non-polyester constituents remaining after dissolution of the polyester-heavy blend feedstock may be treated for dissolution of cellulose to produce liquefied cellulose. Undissolved components such as other fibers, zippers, buttons, and the like, may be collected and re-used or discarded. Additional processing details, conditions and reagents for pretreatment and pulping/dissolution stages are described below.

FIG. 12 illustrates an exemplary overall process flow diagram for treating predominantly cellulosic blended textile input to produce isolated cellulose polymers, identified in FIG. 12 as "Liquefied Cellulose," and isolated polyester polymers, identified in FIG. 12 as "Liquefied Polyester." The liquefied cellulose and polyester products may be suitable for use in a variety of downstream applications, such as fiber production (e.g., textiles, technical fibers and geo-textiles), production of other extrusion and/or constructional manufacturing methods (e.g., 3D printing media, membranes, injection molding media), use as a chemical feedstock for production of biofuels, lubricants and other chemical manufacturing, and for use as food additives, in films, coating, fillers, membranes, packaging, construction materials, non-woven materials, and the like.

FIG. 13 illustrates an exemplary overall process flow diagram for treating predominantly polyester blended textile feed materials to produce liquefied polyester and liquefied cellulosic components suitable for fiber extrusion and including additional processing stages for production of regenerated fibers. FIGS. 14A and 14B schematically illustrate a simplified protocol for processing liquefied cellulose

(FIG. 14A) and liquefied polyester (FIG. 14B) to produce regenerated cellulosic fiber and regenerated polyester fiber, respectively.

#### Fiber Carbonization

In another aspect, methods for carbonizing or graphitizing fibers are disclosed, and carbonized or graphitized fibers are produced. Many types of fibers, such as extruded fibers comprising cellulose derived from biomass and/or textile recycling (as described above), cotton, rayon, lignin, polyacrylonitrile (PAN), acrylic monomers, pitch and other monomeric or polymeric precursors may be used as feed for carbonization. In some embodiments, precursor fibers for carbonization comprise extruded fibers regenerated from post-consumer textile (e.g., cotton) waste. Precursor fibers may be extruded under controlled conditions to produce fibers having a desired size (e.g., diameter) and cross-sectional configuration to accommodate substantial mass losses during the carbonization process and to produce carbonized fibers having desired sizes and configurations.

Cellulose-based fibers generated by treating and dissolving cellulosic-based fabrics and other types of cellulosic feedstocks as described herein may be treated with a precursor and stabilized as feed fiber for carbonization.

Stabilization of regenerated cellulosic fibers prior to carbonization treatment generally involves treatment at a temperature of up to about 400° C. In one embodiment, regenerated cellulosic fibers as described herein are soaked in a dilute acidic bath prior to stabilization and carbonization. In an exemplary embodiment, regenerated cellulosic fibers are treated in a 5% phosphoric acid bath before a stabilization phase (heating to up to 400° C.) prior to a carbonization process. Other types of precursor fibers, as mentioned above, may also be used as feed fibers for carbonization.

In one embodiment, precursor fibers (optionally pretreated with an acid such as phosphoric acid and stabilized by heating at a temperature of up to about 400° C.) are coiled on a rotating rod that can withstand high temperature conditions without degrading, such as a carbon rod that transits a sealed oven or heating zone having zones of increasing temperature along its length. In some embodiments, a rod having a generally cylindrical cross-section may be used; it will be appreciated that rods having square or other polygonal configurations, or oblong, tri-lobal or other configurations may also be used.

In some embodiments, a carbonizing oven temperature may increase from about 400° C. to about 1200° C. or 1500° C. over its length. The atmosphere in the sealed carbonizing oven is preferably inert and non-oxygen-containing, and it preferably contains a gas such as nitrogen or an inert gas.

Gases generated during the carbonizing process (e.g., oxygen) may be evacuated from the carbonizing oven. Appropriate dwell times in the oven depend on a variety of variable factors, including the composition of the precursor fiber, the diameter and structure of the precursor fiber, the rod diameter, the angle of coiling, the length of the oven and dwell time in various zones, and the rod rotational rate. The resulting carbonized fiber coil diameter and fiber density may be engineered to produce desired results, for example, by modifying the precursor material, the coil angle and rod diameter, rod rotational rate, temperature and rate of temperature increase in the carbonizing oven, etc. Carbonized coils may be further processed, such as coated or otherwise treated to impart other desired properties (e.g., chemical, physical, mechanical, etc.), and may be mixed with other fibers in various types of matrices.

Coiled, carbonized fibers produced as described above lose a significant amount of mass during carbonization as a

result of removal of oxygen and other molecules, and generally have a substantially hollow configuration following carbonization. Carbonized fibers have superior insulation properties, are lightweight, and can be engineered to have capillary functions and other surface or mechanical properties. By selecting appropriate precursor fiber compositions, precursor fiber diameters and cross-sectional configurations, coil angles, rod size, shape and rotational rate, and the degree of carbonization (e.g., time in various zones in a carbonization oven, oven temperature and temperature transitions, etc.), carbonized fibers having desired stretch and return on energy parameters may be engineered. Such fibers may be used as microstructures in integrated matrixes that may be incorporated in cushioning or elastic materials, compositions, and the like.

Although the process has been described primarily with reference to using cotton garments and feedstock containing cotton materials and mixed cotton and polyester materials, it will be appreciated that other types of fabrics may be dissolved and regenerated using the same or similar processes to produce regenerated fibers. It will also be appreciated that additional process steps may be employed, as is known in the art, and that equivalent treatment steps may be substituted for those described above.

## EXAMPLES

### Example I

A small-scale experiment was conducted to establish the feasibility of cellulose pulping and fiber regeneration using shredded cotton garment material as a feedstock. The shredded feedstock material was treated with Schweizer's Reagent to form a dissolved pulping solution, and the pulp solution was acidified by treatment with sulfuric acid. Fibers were regenerated as a result of the acidification.

#### Chemical Reactions

1.  $2\text{NaOH}(\text{aq}) + \text{CuSO}_4(\text{aq}) \rightarrow \text{Cu}(\text{OH})_2(\text{s}) + \text{Na}_2\text{SO}_4(\text{aq})$
2.  $\text{Cu}(\text{OH})_2(\text{aq}) \rightarrow \text{Cu}^{2+}(\text{aq}) + 2\text{OH}^-(\text{aq})$
3.  $n\text{ Cu}^{2+}(\text{aq}) + (\text{cellulose})_n + 2n\text{ OH}^- \rightarrow (\text{CuC}_6\text{H}_8\text{O}_5)_n + 2n\text{ H}_2\text{O}$
4. Cellulose is actually dissolved in  $[\text{Cu}(\text{NH}_3)_4](\text{OH})_2$  solution and then regenerated as cotton or rayon when extruded into sulfuric acid.
5. Note: Filtration of  $\text{Cu}(\text{OH})_2$  can be a problem; small amounts of precipitate should be filtered and then combined in one container.

#### Process Instructions

1. Dissolve 25.0 g of  $\text{CuSO}_4 \cdot 5\text{H}_2\text{O}$  in 100 mL distilled water. Heat the water to accelerate the dissolving process.
2. Dissolve 8.0 grams  $\text{NaOH}$  in 200 mL distilled water.
3. Mix the cooled  $\text{NaOH}$  solution with the copper sulfate solution. Collect the resultant gelatinous precipitate of  $\text{Cu}(\text{OH})_2$  by filtration. Wash the precipitate with three 10-mL portions of distilled water. If using 11.0 cm filter paper, several filtrations will be required because of the large amount of precipitate produced.
4. Measure 70 ml concentrated  $\text{NH}_3(\text{aq})$  into a 250-mL Erlenmeyer flask. Shred 10-15 grams cotton garment. Add the  $\text{Cu}(\text{OH})_2$  precipitate carefully along with the filter paper to this flask and stir. This should result in a deep purplish-blue solution of tetraaminecopper(II) hydroxide, referred to as Schweizer's reagent. Stopper the flask and stir periodically for 24 hours or more. Use a magnetic stirrer, if available. One may dip the flask in warm water to speed the process.

5. Take up the contents of the 230-mL Erlenmeyer flask in 10-mL increments in a 10-mL or 50-mL syringe. Squeeze out the contents into a 1000-mL beaker containing 300 mL of 1.6 M sulfuric acid. Be sure that the tip of the syringe or pipet is under the surface of the acid. Crude "thread" forms.

6. The clumps or threads can be washed free of the solution to show the blue-cast white color of the regenerated fibers. Subsequent analysis will demonstrate whether the regenerated fibers have the structure of cotton or rayon.

In alternative schemes, chemical reaction (1), noted above, may be omitted when using copper hydroxide and ammonia reactants to form Schweizer's reagent as follows:



### Example II

Analyses were conducted to compare regenerated cellulosic fibers, processed as described herein, with virgin cotton fibers. Regenerated cellulosic fiber produced as described 25 above was tested using the ASTM D 2256-02 test method for tensile properties of yarns by single-strand method. The regenerated cellulosic fibers exhibited uniform-diameter fiber properties, with the tenacity of cotton and the fineness of silk. Tenacity is a measure of the breaking strength of a fiber divided by the denier. FIG. 11A shows a magnified image of a regenerated cellulosic fiber produced as described above (on the left, labeled Evrnu) and FIG. 11B shows a magnified image of a premium long-staple cotton fiber as tested in Harzallah, Benzina & Drean, 2009 (right-side image, labelled "cotton," reproduced without permission from aforementioned paper). The comparative fiber properties of the regenerated cellulosic fiber produced as described above and the premium long-staple cotton fiber, as reported in the above-mentioned literature reference, are outlined below.

| Fiber Properties                                        | Evrnu                            | Comparison Cotton                                                                                                       |
|---------------------------------------------------------|----------------------------------|-------------------------------------------------------------------------------------------------------------------------|
| Fiber diameter in micrometers (mean/standard deviation) | 20 to 100 (can be customized)    | 226.2/80.3                                                                                                              |
| Tenacity (gf/tex) - mean                                | 21.96                            | 21.01                                                                                                                   |
| Tenacity (gf/tex) - standard dev.                       | 0.64                             | 0.61                                                                                                                    |
| Elongation % - mean                                     | 2 to 4% depends on crystallinity | 8.4%                                                                                                                    |
| Sample size & comment                                   | sample size of 3 fibers          | Cotton #1 sample, tested via the MVI method, is selected from Harzallah, Benzina & Dean 2009, Sample size of 25 fibers. |

55 The tenacity tests indicate that regenerated cellulosic fiber produced as described above has similar strength to the tested cotton, for its diameter. Extrusion allows the diameter (and hence absolute strength of individual fibers) to be tightly controlled.

60 FIG. 11 C shows a magnified cross-sectional image of a regenerated cellulosic fiber produced as described above. Extrusion allows for precision control and consistency in fiber cross-section and length. Regenerated cellulosic fibers produced as described herein may be extruded under various

conditions and to produce different fiber cross-sectional profiles and lengths. In general, regenerated cellulosic fibers produced herein may be extruded just as other manmade fibers and can be prepared as mono, multifilament or stapled in desired length for ring/OE spinning.

## Example III

A small-scale experiment was conducted to establish the feasibility of cellulose pulping and fiber regeneration using shredded cotton garment material as a feedstock and using [EMIM] AcO as a pulping agent. The shredded feedstock material was pretreated, dried to a moisture content of less than 20%, and mixed with [EMIM] AcO in a cellulose dissolution phase. The [EMIM]AcO was about 89% pure, and the pulping phase was maintained at a temperature of from about 85° C. to 95° C. Feedstock loading of approx. 20% was used, with mixing/residence times of from 30 min to 6 hours. The resulting cellulosic pulp was extruded with an air gap in warm water. Regenerated cellulosic fibers having desirable properties were produced.

In the description provided herein, the term "about" means +/-20% of the indicated value or range unless otherwise indicated. The terms "a" and "an," as used herein, refer to one or more of the enumerated components or items. The use of alternative language (e.g., "or") will be understood to mean either one, both or any combination of the alternatives, unless otherwise expressly indicated. The terms "include" and "comprise" and "have" are used interchangeably and each of these terms, and variants thereof, are intended to be construed as being non-limiting.

What is claimed is:

1. A method for producing a composite fiber comprising at least two distinct fiber components, the method comprising:

providing a dissolved cellulosic material;  
providing a second dissolved material; and  
producing a composite fiber by coiling the composite fiber

around a rotating carbon rod with a cylindrical cross-section, the composite fiber having:

a first distinct fiber component comprising the dissolved cellulosic material, the first distinct fiber component having a first partial fiber characteristic and having a first cross-sectional shape, and

a second distinct fiber component comprising the second dissolved material, the second distinct fiber component having a second partial fiber characteristic and having a second cross-sectional shape different from the first cross-sectional shape, wherein the composite fiber has a targeted comfort and performance characteristic and a pre-determined cross-sectional shape and three-dimensional (3D) coiled configuration based on the cylindrical cross-section of the rotating carbon rod, a combination of the first partial fiber characteristic, and the first cross-sectional shape and the second partial fiber characteristic and the second cross-sectional shape.

2. The method of claim 1, wherein the composite fiber is produced by coextruding the first and second distinct fiber components.

3. The method of claim 2, wherein the first distinct fiber component is coextruded as a core fiber and the second distinct fiber components is coextruded as a sheath fiber.

4. The method of claim 2, wherein the second distinct fiber component is coextruded as a core fiber and the first distinct fiber components is coextruded as a sheath fiber.

5. The method of claim 1, wherein the first and second distinct fiber components are coextruded in a side-by-side arrangement.

6. The method of claim 1, wherein the dissolved cellulosic material is produced by treating cellulose-containing feedstock with a dissolving agent.

7. The method of claim 6, further comprising forming a cellulose-containing solid from the cellulose-containing feedstock prior to treatment with the dissolving agent.

8. The method of claim 6, further comprising:  
subjecting the cellulose-containing feedstock to at least one pretreatment stage prior to treatment with the dissolving agent; and  
drying the cellulose-containing feedstock to a moisture content of less than 15% after pretreatment and prior to treatment with the dissolving agent.

9. The method of claim 6, wherein the treatment with the dissolving agent occurs at 60-120° C.

10. The method of claim 6, wherein the dissolving agent comprises

Cu(NH3)4(OH2)(cuoxam); CuH2NCH2CH2NH)2(OH)2 (cuen), Cupriethylenediamine (CED), Ni(NH3)6(OH)2, Cd(H2NCH2CH3NH2)3(OH)2(cadoxen); Zn(H2NCH2CH2NH2)3(OH)2; Fe/3(tartaric acid/\_3NaOH(EWNN); LiOH; Cl3CHO/DMF; (CH2O)x/DMSO; N2O4/DMSO; Li/DMAC(N,N,-dimethylacetamide; LiCl/DMI (N,N,-dimethylimidazolin-dinone); SO2/amine/DMSO; CH3NH2/DMSO; CF3COOH; alkaline Xanthogenation compositions; CS2/NaOH; ZnC12 (<64%); Ca(SCN)3(>50%); Bu (4N+F

3H2O/DMSO; NH4SCN/NH3/water; CO(NH2)2(urea); H2SO4(>52%) (sulfuric acid);

[NMMO] N-methylmorpholine-N-oxide; [AMIM] Cl 1-Allyl-3-methylimidazolium chloride;

[BzPy] Cl Benzylpyridinium chloride; [BMIM] Ace

1-Butyl-3-methylimidazolium acesulphamate;

[BMIM] DBP 1-Butyl-3-methylimidazolium dibutylphosphate;

[BMIM] Cl 1-Butyl-3-methylimidazolium chloride;

[BMIM]PF6 1-Butyl-3-methylimidazolium hexafluorophosphate; [BMIM]BF4 1-Butyl-3-methylimidazolium tetrafluoroborate; [BMPy] Cl 1-Butyl-3-methylpyridinium chloride; [DBNH]AcO 1,8-Diazabicyclo [5.4.0]undec-7-enium acetate; [DBNH]EtCOO 1,8-Diazabicyclo [5.4.0] undec-7-enium propionate; [DMIM] DEP 1,3-Dimethylimidazolium diethylphosphate; [DMIM] DMP 1,3-Dimethylimidazolium dimethylphosphate; [EMBy] DEP 1-Ethyl-3-methylbutylpyridinium diethylphosphate;

[EMIM]AcO 1-Ethyl-3-methylimidazolium acetate;

[EMIM]BR1-Ethyl-3-methylimidazolium bromide;

[EMIM] DBP 1-Ethyl-3-methylimidazolium dibutylphosphate; [EMIM] DEP 1-Ethyl-3-methylimidazolium diethylphosphate;

[EMIM]DMP 1-Ethyl-3-methylimidazolium dimethylphosphate; [EMIM]MeSO4 1-Ethyl-3-methylimidazolium methanesulphonate; [HPy]Cl 1-Hexylpyridinium chloride;

[E(OH) MIM]AcO 1-Hydroxyethyl-3-methylimidazolium acetate; [DBNMe]DMP 1-Methyl-1,8-diazabicyclo [5.4.0]undec-7-enium dimethylphosphate; [P4444]

OH Tetrabutylphosphonium hydroxide; [TMGH]AcO 1,1,3,3-Tetramethylguanidinium acetate;

[TMGH]n-PrCOO 1,1,3,3-Tetramethylguanidinium butyrate; [TMGH]COO 1,1,3,3-Tetramethylguanidinium formate; [TMGH]EtCOO 1,1,3,3-Tetramethyl-

**25**

guanidinium propionate; [P8881]AcO Trioctylmethylphosphonium acetate; HEMA Tris-(2-hydroxyethyl)methylammonium methylsulphate; [DBNMe]DMP 1-Methyl-1,8-diazabicyclo [5.4.0] undec-7-enium dimethylphosphate; Ca, Mg, Na, K, and/or Li hydroxides; and combinations thereof.

**11.** The method of claim **6**, wherein the cellulose-containing feedstock comprises cellulose-containing textiles and garments, post-consumer waste, or combinations thereof.

**12.** The method of claim **1**, wherein the dissolved cellulosic material is provided by:

forming cellulose-containing solid from cellulose-containing feedstock; and

isolating cellulose molecules by treating the cellulose-containing solid with a reagent.

**13.** The method of claim **12**, wherein the forming step comprises the sub-steps comprising

removing, from the cellulose-containing feedstock, a dye, a chemical finish, a contaminant, or a combination thereof; and

pretreating the cellulose-containing feedstock with a swelling agent.

**26**

**14.** The method of claim **13**, wherein the removing step comprises treatment with an oxidative agent, a reducing agent, or both.

**15.** The method of claim **13**, wherein the swelling agent is an ionic solution.

**16.** The method of claim **12**, wherein the reagent disrupts one or more intermolecular hydrogen bonds, thereby converting the at least one cellulose-containing solid to at least one constituent cellulose polymer.

**17.** The method of claim **12**, wherein the reagent is Schweitzer's Reagent.

**18.** The method of claim **12**, wherein the forming step comprises organic solvent treatment with an organic solvent, enzymatic treatment by exposure to an enzyme, or treatment with a swelling agent.

**19.** The method of claim **12**, wherein the cellulose-containing feedstock comprises cellulose-containing textiles and garments, post-consumer waste, or combinations thereof.

**20.** The method of claim **1**, wherein the second dissolved material is carbon-based.

\* \* \* \* \*